



US006393985B1

(12) **United States Patent**  
Tashiro et al.

(10) **Patent No.:** US 6,393,985 B1  
(45) **Date of Patent:** May 28, 2002

(54) **DIRECT DRAWING TYPE LITHOGRAPHIC PRINTING PLATE PRECURSOR**

(75) Inventors: **Hiroshi Tashiro; Eiichi Kato**, both of Shizuoka (JP)

(73) Assignee: **Fuji Photo Co., Ltd.**, Kanagawa (JP)

(\*) Notice: Subject to any disclaimer, the term of this patent is extended or adjusted under 35 U.S.C. 154(b) by 0 days.

(21) Appl. No.: **09/473,501**

(22) Filed: **Dec. 28, 1999**

(30) **Foreign Application Priority Data**

Dec. 28, 1998 (JP) ..... 10-373685  
Dec. 28, 1998 (JP) ..... 10-373686  
Mar. 2, 1999 (JP) ..... 11-054323

(51) **Int. Cl. 7** ..... B41N 1/14

(52) **U.S. Cl.** ..... 101/462, 428/328

(58) **Field of Search** ..... 101/457, 462, 101/463.1, 465, 466, 460; 430/49, 96, 302, 270.1; 428/195, 328

(56) **References Cited**

U.S. PATENT DOCUMENTS

6,019,045 A \* 2/2000 Kato et al. ..... 101/466  
6,183,923 B1 \* 2/2001 Kato et al. ..... 430/96  
6,231,988 B1 \* 5/2001 Kato et al. ..... 428/447  
6,232,034 B1 \* 5/2001 Kasai et al. ..... 430/270.1  
6,258,512 B1 \* 7/2001 Kasai et al. ..... 430/302

\* cited by examiner

*Primary Examiner*—Stephen R. Funk

(74) *Attorney, Agent, or Firm*—Reed Smith LLP

(57) **ABSTRACT**

A direct drawing type lithographic printing plate precursor comprising a water-resistant support having provided thereon an image-receiving layer comprising inorganic particles and a binder resin, wherein the inorganic particles comprise at least one kind of particles selected from: (i) metal oxide particles having an average particle size of from 0.01 to 5  $\mu\text{m}$  and comprising a metal atom selected from Mg, Ba, Ge, Sn, Zn, Pb, La, Zr, V, Cr, Mo, W, Mn, Co, Ni and Cu; (ii) metal hydroxide particles having an average particle size of from 0.01 to 5  $\mu\text{m}$ , the metal hydroxide being represented by the formula (I):



wherein M represents a metal atom selected from Mg, Ba, Al, Ti, Zn, Cu, Ni, Sn, Co, Ge, Fe and La, and x represents a valence of the metal M; and (iii) double oxide particles having an average particle size of from 0.01 to 5  $\mu\text{m}$  and comprising at least one metal atom selected from Mg, Al, Si, Ti, Zr, Cr, V, Mo, Sn, W and Nb, and wherein the binder resin comprises a complex comprising: a resin containing a siloxane bond in which a silicon atom is connected with an oxygen atom; and an organic polymer containing a group capable of forming a hydrogen bond with the resin containing a siloxane bond.

**15 Claims, 4 Drawing Sheets**



FIG. 1



FIG. 2



FIG. 3



FIG. 4



FIG. 5



# DIRECT DRAWING TYPE LITHOGRAPHIC PRINTING PLATE PRECURSOR

## FIELD OF THE INVENTION

The present invention relates to a direct drawing type lithographic printing plate precursor and, more particularly, to a direct drawing type lithographic printing plate precursor capable of providing a printing plate which enables to print a great number of printed matter having clear images free from background stain.

## BACKGROUND OF THE INVENTION

Lithographic printing plate precursors which are mainly used at present in the field of small-scale commercial printing include (1) a direct drawing type lithographic printing plate precursor having a hydrophilic image-receiving layer provided on a water-resistant support, (2) a printing plate precursor having provided on a water-resistant support a lipophilic image-receiving layer comprising zinc oxide, which is converted into a printing plate by undergoing direct drawing image formation and then oil-desensitizing treatment with an oil-desensitizing solution to render the non-image area hydrophilic, (3) a printing plate precursor of an electrophotographic light-sensitive material having provided on a water-resistant support a photoconductive layer comprising photoconductive zinc oxide, which is converted into a printing plate by undergoing image formation and then oil-desensitizing treatment with an oil-desensitizing solution to render the non-image area hydrophilic, and (4) a printing plate precursor of a silver-halide photographic material having a silver halide emulsion layer provided on a water-resistant support.

With the development of office appliances and the expansion of office automation in recent years, it has been desired in the field of printing to adopt an offset printing system wherein a lithographic printing plate is directly prepared from the direct drawing type printing plate precursor (the foregoing (1)) utilizing various image forming means, e.g., an electrophotographic printer, a thermal transfer printer or an ink jet printer without undergoing any other special treatment for conversion into the printing plate.

A conventional direct drawing type lithographic printing plate precursor comprises a support such as paper, having on one surface side thereof an image-receiving layer which is a surface layer provided via an interlayer and on the other surface side thereof a back layer. The interlayer and the back layer are each composed of a water-soluble resin such as PVA or starch, a water-dispersible resin such as a synthetic resin emulsion, and a pigment. The image-receiving layer ordinarily comprises an inorganic pigment, a water-soluble resin and a water resisting agent.

Examples of inorganic pigment used include kaolin, clay, talc, calcium carbonate, silica, titanium oxide, zinc oxide, barium sulfate and alumina.

Examples of water-soluble resin used include polyvinyl alcohol (PVA), modified PVA such as carboxylated PVA, starch and derivatives thereof, cellulose derivatives such as carboxymethyl cellulose and hydroxyethyl cellulose, casein, gelatin, polyvinyl pyrrolidone, vinyl acetate-crotonic acid copolymer, and styrene-maleic acid copolymer.

Examples of water resisting agent used include glyoxal, initial condensates of aminoplasts such as melamine-formaldehyde resin and urea-formaldehyde resin, modified polyamide resins such as methylolated polyamide resin, polyamide-polyamine-epichlorohydrin adduct, polyamide epichlorohydrin resin, and modified polyamide-polyimide resin.

In addition to the above described ingredients, it is known that a cross-linking catalyst such as ammonium chloride or a silane coupling agent can also be used.

Further, it is proposed that as a binder resin used in an image-receiving layer of a direct drawing type lithographic printing plate precursor, a resin having a functional group capable of forming a carboxy group, a hydroxy group, a thiol group, an amino group, a sulfo group or a phosphono group upon decomposition and being previously crosslinked with heat- or light-curing groups included therein is used as described in JP-A-1-226395, JP-A-1-269593 and JP-A-1-288488 (the term "JP-A" as used herein means an "unexamined published Japanese patent application"), a resin having the above-described functional group is used together with a heat- or light-curing resin as described in JP-A-1-226546, JP-A-1-275191 and JP-A-1-309068, or a resin having the above-described functional group is used together with a curing agent as described in JP-A-1-267093, JP-A-1-271292 and JP-A-1-309067, for the purpose of improving hydrophilicity of the non-image area, film strength of the image-receiving layer and printing durability.

It is also proposed that into the image-receiving layer, resin particles having a minute particle size of one  $\mu\text{m}$  or less and containing a hydrophilic group, for example, a carboxy group, a sulfo group or a phosphono group are incorporated as described in JP-A-4-201387 and JP-A-4-223196, or resin particles having a minute particle size and containing a functional group capable of forming the hydrophilic group as described above upon decomposition are incorporated as described in JP-A-4-319491, JP-A-353495, JP-A-5-119545, JP-A-5-58071 and JP-A-5-69684.

However, for improving printing durability of a printing plate obtained by a conventional manner as described above, if the hydrophobicity of the printing plate is enhanced by adding a large amount of the water resisting agent or by using a hydrophobic resin, printing stains due to the decrease in hydrophilicity occur although the printing durability is improved. On the contrary, the enhancement of hydrophilicity results in lowering of the water resistance to cause deterioration of the printing durability.

In particular, when the printing plate is used under a high temperature condition of 30° C. or more, it has a defect that the surface layer thereof is dissolved in dampening water used for offset printing to result in deterioration of the printing durability and occurrence of printing stain. Moreover, since images are directly drawn on an image-receiving layer of a printing plate precursor with oil-based ink in the case of direct drawing type lithography, poor adhesion of the oil-based ink to the image-receiving layer causes falling off of the oil-based ink in the image area during printing, thereby deteriorating the printing durability even if the occurrence of printing stains in the non-image area is prevented because of sufficient hydrophilicity. This problem does not yet come to a satisfactory solution.

On the other hand, a printing plate precursor having a hydrophilic layer containing titanium oxide, polyvinyl alcohol and hydrolyzed tetramethoxysilane or tetraethoxysilane as an image-receiving layer has been proposed as described, for example, in JP-A-3-42679 and JP-A-10-268583. As a result of plate-making of such a printing plate precursor to prepare a printing plate and printing using the printing plate, however, it has been practically found that printing durability of the image is insufficient.

## SUMMARY OF THE INVENTION

The present invention aims to solve these problems which conventional direct drawing type lithographic printing plate precursors are encountered.

Therefore, an object of the present invention is to provide a direct drawing type lithographic printing plate precursor on which neither background stain over an entire surface nor dot-like stain occurs at the plate-making.

Another object of the present invention is to provide a direct drawing type lithographic printing plate precursor capable of forming a printing plate which can provide a great number of printed matter having clear images free from background stain and disappearance or distortion of images.

Other objects and effects of the present invention will become apparent from the following description.

It has been found that these objects of the present invention are accomplished by providing:

a direct drawing type lithographic printing plate precursor comprising a water-resistant support having provided thereon an image-receiving layer comprising inorganic particles and a binder resin,

wherein said inorganic particles comprise at least one kind of particles selected from:

(i) metal oxide particles having an average particle size of from 0.01 to 5  $\mu\text{m}$  and comprising a metal atom selected from Mg, Ba, Ge, Sn, Zn, Pb, La, Zr, V, Cr, Mo, W, Mn, Co, Ni and Cu;

(ii) metal hydroxide particles having an average particle size of from 0.01 to 5  $\mu\text{m}$ , said metal hydroxide being represented by the following formula (I):



wherein M represents a metal atom selected from Mg, Ba, Al, Ti, Zn, Cu, Ni, Sn, Co, Ge, Fe and La, and x represents a valence of said metal M; and

(iii) double oxide particles having an average particle size of from 0.01 to 5  $\mu\text{m}$  and comprising at least one metal atom selected from Mg, Al, Si, Ti, Zr, Cr, V, Mo, Sn, W and Nb, and

wherein said binder resin comprises a complex comprising: a resin containing a siloxane bond in which a silicon atom is connected with an oxygen atom; and an organic polymer containing a group capable of forming a hydrogen bond with said resin containing a siloxane bond.

#### BRIEF DESCRIPTION OF THE ACCOMPANYING DRAWINGS

FIG. 1 is a schematic view showing an example of a device system to which the present invention is applied.

FIG. 2 is a schematic view showing the main part of an ink jet recording device which is utilized for the formation of image on the direct drawing type lithographic printing plate precursor of the present invention.

FIG. 3 is a partially cross sectional view of a head of an ink jet recording device which is utilized for the formation of image on the direct drawing type lithographic printing plate precursor of the present invention.

FIG. 4 is a schematic view showing the main part of a head of another ink jet recording device which is utilized for the formation of image on the direct drawing type lithographic printing plate precursor of the present invention.

FIG. 5 is a schematic view of the head shown in FIG. 4 for explanation.

In these figures, the numerals denote the following members, respectively:

1 Ink jet recording device

2 Lithographic printing plate precursor (Master)

- 3 Computer
- 4 Bus
- 5 Video camera
- 6 Hard disk
- 7 Floppy disk
- 8 Mouse
- 10 Head
- 10a Ejection slit
- 10b Ejection electrode
- 10c Counter electrode
- 11 Oil-based ink
- 101 Upper unit
- 102 Lower unit
- 13 Ink jet recording head
- 14 Body of head
- 15 Meniscus regulation board
- 16 Meniscus regulation board
- 17 Ejection electrode
- 18 Ink groove
- 19 Separator wall
- 20 Ejection part
- 20' Ejection part
- 21 Separator wall
- 22 Tip part of separator wall

#### DETAILED DESCRIPTION OF THE INVENTION

The present invention also includes the following embodiments:

- (1) the direct drawing type lithographic printing plate precursor as described above, wherein the resin containing a siloxane bond, which is present in the image-receiving layer, is a polymer formed by a hydrolysis polymerization condensation reaction of at least one silane compound represented by the following formula (II):



wherein R<sup>0</sup> represents a hydrogen atom, a hydrocarbon group or a heterocyclic group; Y represents a hydrogen atom, a halogen atom, —OR<sup>1</sup>, —OCOR<sup>2</sup> or —N(R<sup>3</sup>)(R<sup>4</sup>) (wherein R<sup>1</sup> and R<sup>2</sup> each represents a hydrocarbon group, and R<sup>3</sup> and R<sup>4</sup>, which may be the same or different, each represents a hydrogen atom or a hydrocarbon group); and n represents 0, 1 or 2, provided that the Si atom is not connected to three or more hydrogen atoms,

- (2) the direct drawing type lithographic printing plate precursor as described above, wherein the image-receiving layer has a surface smoothness of not less than 30 seconds/10 ml in terms of a Bekk smoothness.

The present invention will be described in greater detail below.

- 55 The direct drawing type lithographic printing plate precursor of the present invention comprises a water-resistant support having provided thereon an image-receiving layer having a hydrophilic surface and containing: as inorganic particles, at least one of (i) metal oxide particles having an average particle size of from 0.01 to 5  $\mu\text{m}$  and comprising a specific metal atom, (ii) metal hydroxide particles having an average particle size of from 0.01 to 5  $\mu\text{m}$  and comprising a specific metal atom, and (iii) double oxide particles having an average particle size of from 0.01 to 5  $\mu\text{m}$  and comprising a specific metal atom; and as a binder resin, a complex comprising a resin containing a siloxane bond in which a silicon atom is connected with an oxygen atom and an

organic polymer containing a group capable of forming a hydrogen bond with the resin containing a siloxane bond.

The inorganic particles for use in the image-receiving layer according to the present invention are at least one of those selected from particles of the specific metal oxide, metal hydroxide and double oxide.

The metal oxide for use in the image-receiving layer according to the present invention contains a metal atom selected from Mg, Ba, Ge, Sn, Zn, Pb, La, Zr, V, Cr, Mo, W, Mn, Co, Ni and Cu. Any metal oxide is employed as far as it does not cause a problem regarding to stability and safety of material. The metal oxide containing a metal atom selected from Mg, Ge, Sn, Zn, Pb, Zr, V, Cr, W, Ni and Cu is preferred. With respect to a size of the metal oxide particles, an average particle size of the particles is from 0.01 to 5  $\mu\text{m}$ , preferably from 0.02 to 3  $\mu\text{m}$ . In the above described range, the preferred surface smoothness of the image-receiving layer and the sufficient strength of the image area after the image formation are effected and adhesion of printing ink in the non-image area is prevented.

The metal oxide can be produced according to conventionally known methods as described, for example, in Nippon Kagakukai ed., *Jikken Kagaku Koza 9-Mukikagobutsu no Gosei to Seisei—(Experimental Chemistry Course 9—Synthesis and Purification of Inorganic Compounds—)*, Maruzen (1958) and Kagaku Daijiten Henshu Iinkai ed, *Kagaku Daijiten (Encyclopaedia Chimica)* 3, p. 890 to 949, Kyoritsu Shuppan (1963). The metal oxide particles are also available as commercial products manufactured, for example, by Kanto Kagaku Co., Ltd. and Wako Pure Chemical Industries, Ltd. and described, for example, in Shikizai Kyokai ed., *Shikizai Handbook (Coloring Material Handbook)*, p. 250, Asakura Shoten (1989) and Akira Misuno et al, *Toryo.Ganryou (Paints and Pigments)*, p. 184, Nikkan Kogyo Shinbunsha (1960).

The metal hydroxide for use in the image-receiving layer according to the present invention is represented by formula (I) described above. In formula (I), M preferably represents Al, Ti, Zn, Cu, Ni, Sn or Co. The average particle size of the metal hydroxide particles for use in the present invention is suitably from 0.01 to 5  $\mu\text{m}$ , preferably from 0.02 to 3  $\mu\text{m}$ . In the above described range, the preferred surface smoothness of the image-receiving layer and the sufficient strength of the image area after the image formation are effected and the adhesion of printing ink in the non-image area is prevented.

The metal hydroxide can be produced according to conventionally known methods as described, for example, in Nippon Kagakukai ed., *Jikken Kagaku Koza 9—Mukikagobutsu no Gosei to Seisei—(Experimental Chemistry Course 9—Synthesis and Purification of Inorganic Compounds—)*, Maruzen (1958) and Kagaku Daijiten Henshu Iinkai ed, *Kagaku Daijiten (Encyclopaedia Chimica)* 5, p. 18 to 39, Kyoritsu Shuppan (1963). The metal hydroxide particles are also available as commercial products as described, for example, in Shikizai Kyokai ed., *Shikizai Handbook (Coloring Material Handbook)*, p. 250, Asakura Shoten (1989) and Akira Misuno et al, *Toryo.Ganryou (Paints and Pigments)*, p. 184, Nikkan Kogyo Shinbunsha (1960).

The double oxide for use in the image-receiving layer according to the present invention means a compound of higher order which comprises at least two kinds of oxides and in which the presence of a radical ion of oxygen acid is not recognized in its structure. The double oxide comprising at least three kinds of oxides is sometimes specially designated as a compound oxide. The double oxide used contains at least one metal atom selected from Mg, Al, Si, Ti, Zr, Cr,

V, Mo, Sn, W and Nb, and generally further contains at least one metal atom selected from Li, Ca, Ba, Sr, Bi, Zn, Pb, Co, Mn, Cu, Ni, La and Ge in addition to the above described metal atoms. The double oxides composed of two kinds of metal atoms are preferred.

Any double oxide is employed as far as it does not cause a problem regarding to stability and safety of material. With respect to the size of the double oxide particles, the average particle size of the particles is suitably from 0.01 to 5  $\mu\text{m}$ , preferably from 0.02 to 3  $\mu\text{m}$ . In the above described range, the preferred surface smoothness of the image-receiving layer and the sufficient strength of the image area after the image formation are effected and the adhesion of printing ink in the non-image area is prevented.

The double oxide can be produced according to conventionally known methods as described, for example, in Kozo Tabe, Tetsuro Kiyoyama and Kazuo Fueki ed., *Kinzoku Sankabutsu to Fukugou Sankabutsu (Metal Oxides and Compound Oxides)*, Kodansha (1978), Nippon Kagakukai ed., *Shin-Jikken Kagaku Koza 8—Mukikagobutsu no Gosei I—(New Experimental Chemistry Course 8—Synthesis of Inorganic Compounds I—)*, page 312 to 322, Maruzen (1976) and Norihiko Nakanishi and Naochika Bando ed., *Muki Fine Zairyou no Kagaku (Chemistry of Inorganic Fine Materials)*, p. 28, Sankyo Shuppan (1988). The double oxide particles are also available as commercial products as described, for example, in *Kinzoku Yakuhin Sougo Catalogue (Collective Catalogue of Metallic Reagents)*, 10<sup>th</sup> ed., Soekawa Rikagaku Co., Ltd. (1998).

Specific examples of the double oxide for use in the present invention include metal aluminates, for example,  $\text{M}^1\text{Al}_2\text{O}_4$  or  $\text{M}^1\text{O}.\text{Al}_2\text{O}_3$  (wherein  $\text{M}^1$  represents a metal atom such as Mg, Co, Sr, Cu, Ni or Mn), metal silicate, for example,  $\text{M}^2\text{SiO}_3$  (wherein  $\text{M}^2$  represents a metal atom such as Ca, Ba, Mg, Pb, Zn or Ti), cobalt silicate ( $\text{CoSiO}_4$ ), bismuth silicate ( $\text{Bi}_2\text{O}_3.\text{SiO}_2$ ) or aluminum silicate ( $\text{Al}_2\text{O}_3.\text{SiO}_2$ ), metal titanates, for example,  $\text{M}^3\text{TiO}_3$  or  $\text{M}^3\text{O}.\text{TiO}_2$  (wherein  $\text{M}^3$  represents a metal atom such as Ca, Ba, Sr, Mg, Zn, Co, Pb, Ni or Mn), zirconium titanate ( $\text{ZrO}_2.\text{TiO}_2$ ), aluminum titanate ( $\text{Al}_2\text{TiO}_5$ ) or lanthanum titanate ( $\text{La}_2\text{Ti}_2\text{O}_7$ ), metal zirconate, for example,  $\text{M}^4\text{ZrO}_3$  (wherein  $\text{M}^4$  represents a metal atom such as Ca, Ba, Sr, Mg, Cu, Pb, Ni, Co or Zn), lithium zirconate ( $\text{Li}_2\text{ZrO}_3$ ), aluminum zirconate ( $\text{Al}_2\text{O}_3.3\text{ZrO}_2$ ) or titanium zirconate ( $\text{TiO}_2.\text{ZrO}_2$ ), metal stannate, for example,  $\text{M}^5\text{SnO}_3$  (wherein  $\text{M}^5$  represents a metal atom such as Ca, Ba, Sr, Mg, Cu, Pb or Co) or bismuth stannate ( $\text{Bi}_2\text{Sn}_3\text{O}_3$ ), metal chromate, for example,  $\text{M}^6\text{CrO}_4$  (wherein  $\text{M}^6$  represents a metal atom such as Sr, Pb or Co), metal tungstate, for example,  $\text{M}^7\text{WO}_4$  (wherein  $\text{M}^7$  represents a metal atom such as Ca, Ba, Sr, Co, Mg, Cu, Pb, Ni or Mn), aluminum tungstate ( $\text{Al}_2(\text{WO}_4)_3$  or  $\text{Al}_2\text{O}_3.3\text{WO}_3$ ), zirconium tungstate ( $\text{Zr}(\text{WO}_4)_2$  or  $\text{ZrO}_2.2\text{WO}_3$ ) or bismuth tungstate ( $\text{Bi}_2\text{O}_3.\text{WO}_3$ ), metal molybdate, for example,  $\text{M}^8\text{MoO}_4$  (wherein  $\text{M}^8$  represents a metal atom such as Sr, Co, Pb, Cu, Ba or Ni), metal vanadate, for example,  $\text{M}^9\text{V}_2\text{O}_6$  or  $\text{M}^9\text{O}.\text{V}_2\text{O}_5$ , wherein  $\text{M}^9$  represents a metal atom such as Ca, Mg, Mn, Sr, Cu, Ni or Pb), lead titanate zirconate, barium strontium titanate and basic lead chromate ( $\text{PbCrO}_4.\text{PbO}$ ).

The binder resin for use in the image-receiving layer according to the present invention comprises a complex comprising: a resin containing a siloxane bond in which a silicon atom is connected with an oxygen atom (hereinafter also referred to a siloxane polymer); and an organic polymer containing a group capable of forming a hydrogen bond with the resin containing a siloxane bond. The term “complex comprising a siloxane polymer and an organic polymer” means and includes both a sol substance and a gel substance.

The siloxane polymer means a polymer mainly containing a bond composed of "oxygen atom-silicon atom-oxygen atom". The siloxane polymer preferably contains a hydroxy group in a substituent of the main chain and/or at a terminal of the main chain thereof. The siloxane polymer contains a hydrocarbon group, if desired. Thus, the formation of uniform layer and adhesion of the image area are effectively achieved corresponding to the inorganic particles and the organic polymer used in combination.

The siloxane polymer for use in the present invention is preferably a polymer obtained by a hydrolysis polymerization condensation reaction of the silane compound represented by formula (II) described above. The hydrolysis polymerization condensation reaction is a reaction wherein a hydrolyzable group is repeatedly subjected hydrolysis and condensation under an acidic or basic condition to polymerize, thereby forming a hydroxy group. The silane compounds can be used individually or as a mixture of two or more thereof.

Now, the silane compound represented by formula (II) will be described in more detail below.

In formula (II),  $R^0$  preferably represents a hydrogen atom; a straight chain or branched chain alkyl group having from 1 to 12 carbon atoms (e.g., methyl, ethyl, propyl, butyl, pentyl, hexyl, heptyl, octyl, nonyl, decyl or dodecyl) which may have one or more substituents including, for example, a halogen atom (e.g., chlorine, fluorine or bromine atom), a hydroxy group, a thiol group, a carboxy group, a sulfo group, a cyano group, an epoxy group, an  $-OR'$  group (wherein  $R'$  represents a hydrocarbon group, e.g., methyl, ethyl, propyl, butyl, heptyl, hexyl, octyl, decyl, propenyl, butenyl, hexenyl, octenyl, 2-hydroxyethyl, 3-chloropropyl, 2-cyanoethyl, N,N-dimethylaminoethyl, 2-bromoethyl, 2-(2-methoxyethyl)oxyethyl, 2-methoxy-carbonylethyl, 3-carboxypropyl or benzyl), an  $-OCOR'$  group, a  $-COOR'$  group, a  $-COR'$  group, an  $-N(R'')_2$  group (wherein  $R''$  groups, which may be the same or different, each represents a hydrogen atom or a group same as defined for  $R'$ ), an  $-NHCONHR'$  group, an  $-NHCOOR'$  group, a  $-Si(R')_3$  group, a  $-CONHR'$  group or a  $-NHCO$  group; a straight chain or branched chain alkenyl group having from 2 to 12 carbon atoms (e.g., vinyl, propenyl, butenyl, pentenyl, hexenyl, octenyl, decenyl or dodecenyl) which may have one or more substituents selected from those described for the foregoing alkyl group; an aralkyl group having from 7 to 14 carbon atoms (e.g., benzyl, phenetyl, 3-phenylpropyl, naphthylmethyl or 2-naphthylethyl) which may have one or more substituents selected from those described for the foregoing alkyl group; an alicyclic group having from 5 to 10 carbon atoms (e.g., cyclopentyl, cyclohexyl, 2-cyclohexylethyl, 2-cyclopentylethyl, norbornyl or adamantyl) which may have one or more substituents selected from those described for the foregoing alkyl group; an aryl group having from 6 to 12 carbon atoms (e.g., phenyl or naphthyl) which may have one or more substituents selected from those described for the foregoing alkyl group; or a heterocyclic group which may have a condensed ring, containing at least one atom selected from nitrogen, oxygen and sulfur atoms (examples of the hetero ring including a pyran, furan, thiophene, morpholine, pyrrole, thiazole, oxazole, pyridine, piperidine, pyrrolidone, benzothiazole, benzoxazole, quinoline or tetrahydrofuran ring) which may have one or more substituents selected from those described for the foregoing alkyl group.

In a preferred embodiment, Y in formula (II) represents a halogen atom (e.g., fluorine, chlorine, bromine or iodine), or a group of formula  $-OR^1$ ,  $-OCOR^2$  or  $-NR^3R^4$ .

In the group of  $-OR^1$ ,  $R^1$  represents an aliphatic group having from 1 to 10 carbon atoms which may be substituted (e.g., methyl, ethyl, propyl, butyl, pentyl, hexyl, heptyl, octyl, nonyl, decyl, propenyl, butenyl, heptenyl, hexenyl, octenyl, decenyl, 2-hydroxyethyl, 2-hydroxypropyl, 2-methoxyethyl, 2-(methoxyethoxyethyl, 2-(N,N-diethylamino)ethyl, 2-methoxypropyl, 2-cyanoethyl, 3-methoxypropyl, 2-chloroethyl, cyclohexyl, cyclopentyl, cyclooctyl, chlorocyclohexyl, methoxycyclohexyl, benzyl, phenetyl, dimethoxybenzyl, methylbenzyl or bromobenzyl).

In the group of  $-OCOR^2$ ,  $R^2$  represents an aliphatic group as defined for  $R^1$ , or an aromatic group having from 6 to 12 carbon atoms which may be substituted (e.g., aryl groups as described for the forgoing  $R^0$ ).

In the group of  $-NR^3R^4$ ,  $R^3$  and  $R^4$ , which may be the same or different, each represents a hydrogen atom or an aliphatic group having from 1 to 10 carbon atoms which may be substituted (e.g., aliphatic groups as described for  $R^1$  in the foregoing group  $-OR^1$ ). More preferably, the total number of carbon atoms contained in  $R^3$  and  $R^4$  are 16 or less.

Specific examples of the silane compound represented by formula (II) include, but not limited to, methyltrichlorosilane, methyltribromosilane, 25 methyltrimethoxysilane, methyltriethoxysilane, methyltriisopropoxysilane, methyltri(tert-butoxy)ilane, ethyltrichlorosilane, ethyltribromosilane, ethyltrimethoxysilane, ethyltriethoxysilane, ethyltriisopropoxysilane, ethyltri(tert-butoxy)ilane, n-propyltrichlorosilane, n-propyltribromosilane, n-propyltrimethoxysilane, n-propyltriethoxysilane, n-propyltriisopropoxysilane, n-propyltri(tert-butoxy)ilane, n-hexyltrichlorosilane, n-hexyltribromosilane, n-hexyltrimethoxysilane, n-hexyltriethoxysilane, 35 n-hexyltriisopropoxysilane, n-hexyltri(tert-butoxy)ilane, n-decyltrichlorosilane, n-decyltribromosilane, n-decyltrimethoxysilane, n-decyltriethoxysilane, n-decyltriisopropoxysilane, n-decyltri(tert-butoxy)ilane, n-octadecyltrichlorosilane, n-octadecyltribromosilane, n-octadecyltrimethoxysilane, n-octadecyltriethoxysilane, 40 n-octadecyltriisopropoxysilane, n-octadecyltri(tert-butoxy)ilane, phenyltrichlorosilane, phenyltribromosilane, phenyltrimethoxysilane, phenyltriethoxysilane, phenyltriisopropoxysilane, phenyltri(tert-butoxy)ilane, tetrachlorosilane, tetrabromosilane, tetramethoxysilane, tetraethoxysilane, tetraisopropoxysilane, tetrabutoxysilane, dimethoxydiethoxysilane, dimethyldichlorosilane, dimethyldibromosilane, dimethyldimethoxysilane, dimethyldiethoxysilane, diphenyldichlorosilane, 45 diphenyldibromosilane, diphenyldimethoxysilane, diphenyldiethoxysilane, phenylmethyldichlorosilane, phenylmethyldibromosilane, phenylmethyldimethoxysilane, phenylmethyldiethoxysilane, triethoxyhydrosilane, tribromohydrosilane, trimethoxyhydrosilane, triisopropoxyhydrosilane, tri(tert-butoxy)hydrosilane, vinyltrichlorosilane, vinyltribromosilane, vinyltrimethoxysilane, vinyltriethoxysilane, vinyltriisopropoxysilane, vinyltri(tert-butoxy)ilane, 50 trifluoropropyltrichlorosilane, trifluoropropyltribromosilane, trifluoropropyltrimethoxysilane, trifluoropropyltriethoxysilane, trifluoropropyltriisopropoxysilane, trifluoropropyltri(tert-butoxy)ilane,  $\gamma$ -glycidoxypropylmethyldimethoxysilane,  $\gamma$ -glycidoxypropylmethyldiethoxysilane,  $\gamma$ -glycidoxypropyltrimethoxysilane,

$\gamma$ -glycidoxypolypropyltriethoxysilane,  
 $\gamma$ -glycidoxypolytriisopropoxysilane,  $\gamma$ -glycidoxypolypropyltri(tert-butoxy)silane,  
 $\gamma$ -methacryloxypropylmethyldimethoxysilane,  
 $\gamma$ -methacryloxypropylmethyldiethoxysilane,  
 $\gamma$ -methacryloxypropyltrimethoxysilane,  
 $\gamma$ -methacryloxypropyltriisopropoxysilane,  
 $\gamma$ -methacryloxypropyltri(tert-butoxy)silane,  
 $\gamma$ -aminopropylmethyldimethoxysilane,  
 $\gamma$ -aminopropylmethyldiethoxysilane,  
 $\gamma$ -aminopropyltrimethoxysilane,  
 $\gamma$ -aminopropyltriethoxysilane,  
 $\gamma$ -aminopropyltriisopropoxysilane,  $\gamma$ -aminopropyltri(tert-butoxy)silane,  $\gamma$ -mercaptopropylmethyldimethoxysilane,  
 $\gamma$ -mercaptopropylmethyldiethoxysilane,  
 $\gamma$ -mercaptopropyltriethoxysilane,  
 $\gamma$ -mercaptopropyltriisopropoxysilane,  $\gamma$ -mercaptopropyltri(tert-butoxy)silane,  $\beta$ -(3,4-epoxycyclohexyl)ethyltrimethoxysilane and  $\beta$ -(3,4-epoxycyclohexyl)ethyltriethoxysilane.

In combination with the silane compound represented by formula (II) which is used for the formation of the image-receiving layer according to the present invention, a metallic compound capable of forming film by a sol-gel method such as Ti, Zn, Sn, Zr or Al compound can be employed. Specific examples of the metallic compound usable in combination include  $Ti(O^{R^5})_4$  (wherein  $R^5$  represents an alkyl group such as methyl, ethyl, propyl, butyl, pentyl, or hexyl),  $TiCl_4$ ,  $Zn(O^{R^5})_2$ ,  $Zn(CH_3COCHCOCH_3)_2$ ,  $Sn(O^{R^5})_4$ ,  $Sn(CH_3COCHCOCH_3)_4$ ,  $Sn(OCO^{R^5})_4$ ,  $SnCl_4$ ,  $Zr(O^{R^5})_4$ ,  $Zr(CH_3COCHCOCH_3)_4$  and  $Al(O^{R^5})_3$ .

Now, the organic polymer for use in the present invention will be described in more detail below.

The organic polymer contains a group capable of forming a hydrogen bond with the resin containing a siloxane bond as described above. The group capable of forming a hydrogen bond with the resin containing a siloxane bond (hereinafter also referred to as specific bond-forming group) preferably includes an amido bond (including a carbon-amido bond and a sulfonamido bond), a urethane bond, a ureido bond and a hydroxy group.

The organic polymer contains at least one specific bond-forming group in a main chain and/or a side chain thereof as a repeating unit component. The organic polymer preferably includes a polymer containing, as a repeating unit component, a component having at least one bond selected from  $-N(R^{11})CO-$ ,  $-N(R^{11})S_2O-$ ,  $-NHCONH-$  and  $-NHCOO-$  in the main chain or side chain thereof, and a polymer containing, as a repeating unit component, a component having a hydroxy group. In the above-described amido bonds,  $R^{11}$  represents a hydrogen atom or an organic residue, and the organic residue includes the hydrocarbon group and heterocyclic group represented by  $R^0$  in formula (II).

The organic polymer containing the specific bond in its main chain according to the present invention includes an amide resin having the  $-N(R^{11})CO-$  or  $-N(R^{11})SO_2-$  bond, a ureido resin having the  $-NHCONH-$  bond, and a urethane resin having the  $-NHCOO-$  bond.

As diamines and dicarboxylic acids used for preparation of the amide resins, diisocyanates used for preparation of the ureido resins and diols used for preparation of the urethane resins, compounds described, for example, in Kobunshi Gakkai ed., *Kobunshi Data Handbook—Kisohen—* (*Polymer Data Handbook, Fundamental Volume*), Chapter I, Baifukan (1986), Shinzo Yamashita and Tosuke Kaneko ed.,

*Kakyozi Handbook (Handbook of Cross-linking Agents)*, Taiseisha (1981).

Other examples of the polymer containing the amido bond include a polymer containing a repeating unit represented by formula (III) shown below, N-acylated polyalkyleneimine, and polyvinylpyrrolidone and derivatives thereof.



wherein,  $Z^1$  represents  $-\text{CO}-$ ,  $-\text{CS}-$  or  $-\text{SO}_2-$ ;  $R^{20}$  represents a hydrogen atom, a hydrocarbon group or a heterocyclic group (the hydrocarbon group and heterocyclic group having the same meanings as those defined for  $R^0$  in formula (I), respectively);  $r^1$  represents hydrogen atom or an alkyl group having from 1 to 6 carbon atoms (e.g., methyl, ethyl, propyl, butyl, pentyl or hexyl), and a plurality of  $r^1$  groups may be the same or different; and  $p$  represents an integer of 2 or 3.

Among the polymers containing a repeating unit represented by formula (III), a polymer wherein  $Z^1$  represents  $-\text{CO}-$  and  $p$  is 2 can be obtained by ring-opening polymerization of oxazoline which may be substituted in the presence of a catalyst. The catalyst which can be used includes a sulfuric ester or sulfonic ester (e.g., dimethyl sulfate or an alkyl p-toluenesulfonate), an alkyl halide (e.g., an alkyl iodide such as methyl iodide), a fluorinated metallic compound of Friedel-Crafts catalyst, and an acid (e.g., sulfuric acid, hydrogen iodide or p-toluenesulfonic acid) or an oxazolinium salt thereof formed from the acid and oxazoline.

The polymer may be a homopolymer or a copolymer. The polymer also includes a graft polymer containing the units derived from oxazoline in its graft portion.

Specific examples of the oxazoline include 2-oxazoline, 2-methyl-2-oxazoline, 2-ethyl-2-oxazoline, 2-propyl-2-oxazoline, 2-isopropyl-2-oxazoline, 2-butyl-2-oxazoline, 2-dichloromethyl-2-oxazoline, 2-trichloromethyl-2-oxazoline, 2-pentafluoroethyl-2-oxazoline, 2-phenyl-2-oxazoline, 2-methoxycarbonylethyl-2-oxazoline, 2-(4-methylphenyl)-2-oxazoline, and 2-(4-chlorophenyl)-2-oxazoline. Preferred examples of the oxazoline include 2-oxazoline, 2-methyl-2-oxazoline, 2-ethyl-2-oxazoline. The oxazolines may be employed individually or as a mixture of two or more thereof.

Other polymers containing a repeating unit represented by formula (III) are also obtained in the same manner as described above except for using thiazoline, 4,5-dihydro-1,3-oxazine or 4,5-dihydro-1,3-thiazine in place of oxazoline.

The N-acylated polyalkyleneimine includes a carboxylic amide compound containing an  $-N(\text{CO---}R^{20})-$  bond (wherein  $R^{20}$  has the same meaning as defined above) obtained by a polymer reaction of polyalkyleneimine with a carboxylic halide and a sulfonamide compound containing an  $-N(\text{SO}_2---R^{20})-$  bond obtained by a polymer reaction of polyalkyleneimine with a sulfonyl halide.

The organic polymer containing the specific bond in the side chain thereof according to the present invention includes a polymer containing as the main component, a component having at least one bond selected from the specific bonds.

Specific examples of the component having the specific bond include repeating units derived from acrylamide, methacrylamide, crotonamide and vinyl acetamide, and the

11

repeating units shown below, but the present invention should not be construed as being limited thereto.



a<sup>1</sup>: —H, —CH<sub>3</sub>  
 1<sub>1</sub>: an integer from 1 to 4  
 T<sup>0</sup>: —H, —CH<sub>3</sub>, —(CH<sub>2</sub>)<sub>2</sub>OCH<sub>3</sub>,  
 —(CH<sub>2</sub>)<sub>2</sub>N(CH<sub>3</sub>)<sub>2</sub>



$l_2$ : 0 or 1  
 $L^0$ :  $\text{---C}_{n1}\text{H}_{2n1+1}$   
 (n<sub>1</sub>: an integer from 1 to 4)  
 $\text{---}(\text{CH}_2)_2\text{OCH}_3$ ,  $\text{---}(\text{CH}_2)_3\text{N}(\text{CH}_3)_2$   
 $\text{---CH}_2\text{C}_6\text{H}_5$ ,  $\text{---}(\text{CH}_2)_{n1}\text{OH}$



$l_3$ : 0, 1 or 2



12

-continued

(10)



$$(2) \quad ^{15} \quad L^1: \begin{array}{c} L^1 \\ | \\ \text{---H, ---L}^0 \\ | \\ \text{---(CH}_2\text{)}_{l_1}\text{---CONH}_2 \end{array}$$



25 



$$(4) \quad (C_{11}H_{22})_2 \text{OOCNHC}_n\text{H}_2\text{C}_{2n+1} \quad (15)$$



(16)



The organic polymer containing a hydroxy group according to the present invention may be any of natural water-soluble polymers, semisynthetic water-soluble polymers and synthetic water-soluble polymers, and include those described, for example, in Munio Kotake supervised, *Daiyukikagaku 19—Tennen Koubunshi Kagoubutsu I (Grand Organic Chemistry 19—Natural Polymer Compounds I)*, Asakura Shoten (1960), Keiei Kaihatsu Center Shuppanbu ed., *Suiyousei Koubunshi Mizubunsangata Jushi Sougogijutsu (Water-Soluble Polymers. Agueous Dispersion Type Resins; Collective Technical Data)*, Keiei Kaihatsu Center Shuppanbu (1981), Sinji Nagatomo, *Shin-Suiyousei Polymer no Oyou to Shijo (New Applications and Market of Water-Soluble Polymers)*, CMC (1988), and *Kinousei Cel lulose no Kaihatsu (Development of Functional Cellulose)*, CMC (1985).

Specific examples of the natural and semisynthetic water-soluble polymers include cellulose, cellulose derivatives (e.g., cellulose esters such as cellulose nitrate, cellulose 65 sulfate, cellulose acetate, cellulose propionate, cellulose succinate, cellulose butyrate, cellulose acetate succinate, cellulose acetate butyrate or cellulose acetate phthalate; and

cellulose ethers such as methylcellulose, ethylcellulose, cyanoethylcellulose, carboxymethylcellulose, hydroxyethylcellulose, hydroxypropylcellulose, ethyl hydroxyethylcellulose, hydroxypropyl methylcellulose or carboxymethyl hydroxyethylcellulose), starch, starch derivatives (e.g., oxidized starch, esterified starch including those esterified with an acid such as nitric acid, sulfuric acid, phosphoric acid, acetic acid, propionic acid, butyric acid or succinic acid; and etherified starch such as methylated starch, ethylated starch, cyanoethylated starch, hydroxyalkylated starch or carboxymethylated starch), alginic acid, pectin, carrageenan, tamarind gum, natural rubber (e.g., gum arabic, guar gum, locust bean gum, tragacanth gum or xanthane gum), pullulan, dextran, casein, gelatin, chitin and chitosan.

Specific examples of the synthetic water-soluble polymer include polyvinyl alcohol, polyalkylene glycols (e.g., polyethylene glycol, polypropylene glycol or ethylene glycol/propylene glycol copolymers), allyl alcohol copolymers, homopolymers or copolymers of acrylate or methacrylate containing at least one hydroxy group (examples of ester portion including a 2-hydroxyethyl, 3-hydroxypropyl, 2,3-dihydroxypropyl, 3-hydroxy-2-hydroxymethyl-2-methylpropyl, 3-hydroxy-2-di(hydroxymethyl)propyl, polyoxyethylene and polyoxypropylene group), homopolymers or copolymers of N-substituted acrylamide or methacrylamide containing at least one hydroxy group (examples of N-substituent including a monomethylol, 2-hydroxyethyl, 3-hydroxypropyl, 1,1-bis(hydroxymethyl)ethyl and 2,3,4,5,6-pentahydroxypentyl group). However, the synthetic water-soluble polymer is not particularly limited as long as it contains at least one hydroxy group in the side chain substituent of the repeating unit thereof.

The weight average molecular weight of the organic polymer constituting the complex for use in the image-receiving layer according to the present invention is preferably from  $1\times 10^3$  to  $1\times 10^6$ , more preferably from  $5\times 10^3$  to  $4\times 10^5$ .

In the complex comprising a siloxane polymer and an organic polymer according to the present invention, the ratio of the siloxane polymer to the organic polymer can be selected from a wide range, and the weight ratio of the siloxane polymer/organic polymer is preferably from 10/90 to 90/10, more preferably from 20/80 to 80/20.

In such a range, the desired film-strength and water-resistance of the image-receiving layer to dampening water during printing are advantageously effected.

The binder resin comprising the complex of the organic polymer and the inorganic polymer according to the present invention forms a uniform organic/inorganic hybrid by means of the function of hydrogen bonds generated between hydroxy groups of the siloxane polymer produced by the hydrolysis polymerization condensation of the silane compounds as described above and the above described specific bond-forming groups in the organic polymer and is microscopically homogeneous without the occurrence of phase separation to well maintain affinity between the siloxane polymer and the organic polymer. Also, it is believed that the affinity between the siloxane polymer and the organic polymer is more improved due to the function of the hydrocarbon group included in the siloxane polymer. Further, the complex of the siloxane polymer and the organic polymer is excellent in a film-forming property.

The complex of the resins can be prepared by subjecting the silane compound to the hydrolysis polymerization condensation and then mixing with the organic polymer, or by conducting the hydrolysis polymerization condensation of the silane compound in the presence of the organic polymer.

Preferably, the complex of the organic polymer and the inorganic polymer according to the present invention is prepared by conducting the hydrolysis polymerization condensation of the silane compound in the presence of the organic polymer according to a sol-gel method. In the complex of the organic polymer and the inorganic polymer thus prepared, the organic polymer is uniformly dispersed in a matrix (i.e., three-dimensional micro-network structure of inorganic oxide) of gel prepared by the hydrolysis polymerization condensation of the silane compound.

The sol-gel method in the present invention may be performed according to any of conventionally well-known sol-gel methods. More specifically, it is conducted with reference to methods described in detail, for example, in

15 *Sol-Gel-ho nigoru Hakumaku Coating Gijutsu (Thin Film Coating Technology by Sol-Gel Method)*, Gijutsujoho Kyokai (1995), Sumio Sakibana, *Sol-Gel-ho no Kagaku (Science of Sol-Gel Method)*, Agne Shofusha (1988), and Seki Hirashima, *Saishin Sol-Gel-ho nigoru Kinosei Hakumaku 20 Sakusei Gijutsu (Latest Technology of Functional Thin Film Formation by Sol-Gel Method)*, Sogo Gijutsu Center (1992).

In a coating solution for the image-receiving layer, an aqueous solvent is preferably used. A water-soluble solvent is also employed together therewith in order to prevent the occurrence of precipitation during the preparation of coating solution, thereby forming a homogenous solution. Examples of such a water-soluble solvent include an alcohol (such as methanol, ethanol, propyl alcohol, ethylene glycol, diethylene glycol, propylene glycol, dipropylene glycol, ethylene glycol monomethyl ether, propylene glycol monomethyl ether and ethylene glycol monoethyl ether), an ether (such as tetrahydrofuran, ethylene glycol dimethyl ether, propylene glycol dimethyl ether and tetrahydrofuran), a ketone (such as acetone, methyl ethyl ketone and acetylacetone), an ester (such as methyl acetate and ethylene glycol monomethylmonoacetate) and an amide (such as formamide, N-methylformamide, pyrrolidone and N-methylpyrrolidone). These solvents may be used individually or as a mixture of two or more thereof.

In the coating solution, it is preferred to further use an acidic or basic catalyst for the purpose of accelerating the hydrolysis and polymerization condensation reaction of the silane compound represented by formula (II).

The catalyst used for the above purpose is an acidic or basic compound itself or an acidic or basic compound dissolved in a solvent, such as water or an alcohol (hereinafter referred to as an acidic catalyst or a basic catalyst respectively). The concentration of the catalyst is not particularly limited, and the high catalyst concentration tends to increase the hydrolysis speed and the polymerization condensation speed. However, since the basic catalyst used in a high concentration may cause precipitation in the sol solution, it is desirable that the basic catalyst concentration be not higher than one normal (1N), as the concentration in the aqueous solution.

The acidic catalyst or the basic catalyst for use in the invention has no particular restriction as to the species. In a case where the use of a catalyst in a high concentration is required, however, a catalyst constituted of elements which leave no residue in its crystal grains obtained after sintering is preferred. Suitable examples of the acidic catalyst include a hydrogen halide (e.g., hydrogen chloride), nitric acid, sulfuric acid, sulfurous acid, hydrogen sulfide, perchloric acid, hydrogen peroxide, carbonic acid, a carboxylic acid (e.g., formic acid or acetic acid), a substituted carboxylic acid (e.g., an acid represented by formula of  $RCOOH$  wherein R is an element or a substituent other than —H and

$\text{CH}_3$ —), and a sulfonic acid (e.g., benzenesulfonic acid). Suitable examples of the basic catalyst include an ammoniacal base (e.g., aqueous ammonia) and an amine (e.g., ethylamine or aniline).

In addition to the above described components, the image-receiving layer according to the present invention may contain other ingredients.

Examples of other ingredients include inorganic pigment particles other than the specific metal oxide, metal hydroxide and double oxide particles. Examples of such an inorganic pigment include silica, alumina, kaolin, clay, titanium oxide, calcium carbonate, barium carbonate, calcium sulfate, barium sulfate and magnesium carbonate. Such inorganic pigment particles are used in a proportion of preferably not higher than 40 parts by weight, more preferably not higher than 20 parts by weight, based on 100 parts by weight of the metal oxide, metal hydroxide and double oxide particles used in accordance with the present invention.

As for the ratio of the binder resin and the pigment particles (including the metal oxide, metal hydroxide and double oxide particles according to the present invention and other inorganic pigment particles used, if desired) in the image-receiving layer, the amount of the binder resin is preferably from 8 to 50 parts by weight, more preferably from 10 to 30 parts by weight based on 100 parts by weight of the pigment particles. In such a range, the effects of the present invention are efficiently achieved, and the good film-strength of the image-receiving layer can be retained and the good hydrophilicity in the non-image area can be maintained during printing.

Also, the images firmly adhere to the image-receiving layer and the printing plate exhibits good printing durability. Specifically, disappearance of image does not occur after printing a large number of sheets.

To the image-receiving layer, a cross-linking agent may be added for further increasing the film-strength thereof.

The cross-linking agent usable herein include compounds ordinarily used as cross-linking agent. Specifically, such compounds as described, e.g., in Shinzo Yamashita and Tosuke Kaneko ed., *Kakyozai Handbook (Handbook of Cross-linking Agents)*, Taiseisha (1981) and Kobunshi Gakkaishi ed., *Kobunshi Data Handbook—Kisohen—(Polymer Data Handbook, Fundamental Volume)*, Baifukan (1986).

Examples of the cross-linking agent which can be used include ammonium chloride, metal ions, organic peroxides, polyisocyanate compounds (e.g., toluylene diisocyanate, diphenylmethane diisocyanate, triphenylmethane triisocyanate, polymethylene phenylisocyanate, hexamethylene diisocyanate, isophorone diisocyanate, or high molecular polyisocyanate), polyol compounds (e.g., 1,4-butanediol, polyoxypropylene glycol, polyoxyethylene glycol, or 1,1,1-trimethylolpropane), polyamine compounds (e.g., ethylenediamine,  $\gamma$ -hydroxypropylated ethylenediamine, phenylenediamine, hexamethylenediamine, N-aminoethylpiperazine, or modified aliphatic polyamines), polyepoxy group-containing compounds and epoxy resins (e.g., compounds described in Hiroshi Kakiuchi, *Shin Epoxy Jushi (New Epoxy Resins)*, Shokodo (1985), and Kuniyuki Hashimoto, *Epoxy Jushi (Epoxy Resins)*, Nikkan Kogyo Shinbunsha (1969)), melamine resins (e.g., compounds described in Ichiro Miwa & Hideo Matsunaga, *Urea.Melamine Jushi (Urea.Melamine Resins)*, Nikkan Kogyo Shinbunsha (1969)), and poly(meth)acrylate compounds (e.g., compounds described in Makoto Ogawara, Takeo Saegusa & Toshinobu Higashimura, *Oligomer (Oligomers)*, Kodansha (1976), and Eizo Omori,

*Kinousei Acryl Kei Jushi (Functional Acrylic Resins)*, Techno System (1985)).

The coating solution for the image-receiving layer is coated on a water-resistant support using any of conventionally well-known coating methods, and dried to form the image-receiving layer.

The thickness of the image-receiving layer thus formed is preferably from 0.2 to 10  $\mu\text{m}$ , more preferably from 0.5 to 8  $\mu\text{m}$ . In such a thickness range, the layer formed can have a uniform thickness and sufficient film-strength.

The image-receiving layer according to the present invention preferably has a surface smoothness of not less than 30 (sec/10 ml) in terms of a Bekk smoothness.

The term "Bekk smoothness" as used herein means a Bekk smoothness degree measured by a Bekk smoothness tester. In the Bekk smoothness tester, a sample piece is pressed against a circular glass plate having a highly smooth finish and a hole at the center while applying thereto a definite pressure (1 kg/cm<sup>2</sup>), and a definite volume (10 ml) of air is forced to pass between the sample piece and the glass surface under reduced pressure. Under this condition, a time (expressed in second) required for the air passage is measured.

In a case where images are formed on the lithographic printing plate precursor by means of an electrophotographic printer, an appropriate range of the Bekk smoothness depends on whether toner used in the electrophotographic printer is dry toner or liquid toner.

More specifically, in the case of using dry toner in the electrophotographic printer, it is desirable that the Bekk smoothness of the image-receiving layer surface be preferably from 30 to 200 (sec/10 ml), more preferably from 50 to 150 (sec/10 ml). In the above described range, the attachment of scattered toner to the non-image area (occurrence of background stain) is prevented and the toner adheres uniformly and firmly to the image area in the process of transferring and fixing the toner image to the printing plate precursor, whereby satisfactory reproduction of fine lines and fine letters and uniformity in the solid image area can be achieved.

In the case of using liquid toner in the electrophotographic printer, it is desirable for the image-receiving layer surface to have the Bekk smoothness of not less than 30 (sec/10 ml), and the toner images transferred and fixed thereto can have better quality the higher the Bekk smoothness is. Specifically, the range thereof is preferably from 150 to 3,000 (sec/10 ml), more preferably from 500 to 2,500 (sec/10 ml).

In a case where images are formed by means of an ink jet printer or a thermal transfer printer, the Bekk smoothness of the lithographic printing plate precursor surface is preferably in the range described above for the case of using liquid developer in the electrophotographic printer.

In the above described range, highly accurate toner images such as fine lines, fine letters or dots can be transferred faithfully to the image-receiving layer, and fixed thereto so firmly as to ensure sufficient strength in the image area.

It is more preferred that the surface of the image-receiving layer has high protrusions densely. More specifically, the image-receiving layer preferably has an average surface center roughness (SRa) defined in ISO-468 in the range of from 1.3 to 3.5  $\mu\text{m}$ , and an average wavelength (S $\lambda$ a), which indicates the density of the surface roughness, of not more than 50  $\mu\text{m}$ . More preferably, the SRa is in the range of from 1.35 to 2.5  $\mu\text{m}$ , and the S $\lambda$ a is not more than 45  $\mu\text{m}$ . It is believed that the adhesion of scattered toner to the non-

image area after plate-making by electrophotography and spreading of adhered toner during fixing can be prevented owing to the use of the image-receiving layer having the above described surface unevenness.

Now, the water-resistant support which can be used in the present invention will be described in more detail below.

Examples of the water-resistant support for use in the invention include an aluminum plate, a zinc plate, a bimetal plate such as a copper-aluminum plate, a copper-stainless steel plate or a chromium-copper plate, and a trimetal plate such as a chromium-copper-aluminum plate, chromium-lead-iron plate or a chromium-copper-stainless steel plate, which each has a thickness of preferably from 0.1 to 3 mm, more preferably from 0.1 to 1 mm. Also, paper subjected to water-resistant treatment, paper laminated with a plastic film or a metal foil, and a plastic film each preferably having a thickness of from 80 to 200  $\mu\text{m}$  are employed.

The water-resistant support has preferably a highly smooth surface. Specifically, it is desirable for the support used in the present invention that the Bekk smoothness of the surface which contacts with the image-receiving layer be adjusted to preferably at least 300 (sec/10 ml), more preferably from 900 to 3,000 (sec/10 ml), yet more preferably from 1,000 to 3,000 (sec/10 ml). By controlling the Bekk smoothness of the surface contacting the image-receiving layer to at least 300 sec/10 ml, the image reproducibility and the printing durability can be more improved. As such improving effects can be obtained even when the image-receiving layer provided thereon has the same surface smoothness, the increase in the smoothness of the support surface is considered to improve the adhesion between the image area and the image-receiving layer.

The Bekk smoothness of the surface of the support can be measured in the same manner as described with respect to the image-receiving layer.

The expression "highly smooth surface of the water-resistant support" as used herein means a surface coated directly with the image-receiving layer. In other words, when the support has an under and/or overcoat layer, e.g., a conductive layer described below, the highly smooth surface denotes the surface of the under and/or overcoat layer.

Thus, the surface condition of the image-receiving layer can be controlled and fully kept without receiving the influence of surface roughness of the support used. As a result, it becomes possible to further improve the image quality.

The adjustment of the surface smoothness to the above described range can be made using various well-known methods. For instance, the Bekk smoothness of support surface can be adjusted by coating a substrate with a resin using a melt adhesion method, or by using a strengthened calender method utilizing highly smooth heated rollers.

The lithographic printing plate precursor according to the present invention can be preferably used as a printing plate precursor for forming images on the image-receiving layer provided on the water-resistant support with an electrophotographic recording system or an electrostatic ejection type ink jet recording system wherein oil-based ink is ejected utilizing an electrostatic field. The lithographic printing plate thus-prepared can provide a great number of printed matter having clear images.

In the case of utilizing the electrophotographic recording system to form images, transfer of toner images to a material to be transferred in the electrophotographic process is usually carried out electrostatically. In the above case, it is preferred that the water-resistant support is electrically conductive. Specifically, the specific electric resistance of the

water-resistant support is preferably from  $10^4$  to  $10^{13}$   $\Omega\text{-cm}$ , more preferably from  $10^7$  to  $10^{12}$   $\Omega\text{-cm}$ . By adjusting the specific electric resistance to the above described range, blur and distortion of the transferred image and stain due to adhesion of toner to the non-image area can be restrained to a practically acceptable extent, so that the images of good quality can be obtained.

It is desirable for the water-resistant support used in the electrostatic ejection type ink jet recording system to have electric conductivity. At least in the part just under the image-receiving layer, the support has the specific electric resistance of preferably not more than  $10^{10}$   $\Omega\text{-cm}$ . For the water-resistant support as a whole, the specific electric resistance is preferably  $10^{10}$   $\Omega\text{-cm}$  or below, and more preferably  $10^8$   $\Omega\text{-cm}$  or below. The value may be infinitely close to zero.

The electric conductivity as described above can be conferred on the support in the part just under the image-receiving layer, e.g., by coating a substrate such as paper or a film with a layer comprising an electrically conductive filler such as carbon black and a binder, by sticking a metal foil on a substrate, or by vapor-evaporating a metallic film onto a substrate.

On the other hand, examples of the support that is electrically conductive as the whole include electrically conductive paper impregnated with sodium chloride, a plastic film in which an electrically conductive filler such as carbon black is mixed, and a metal plate such as an aluminum plate.

In the above described range of electric conductivity, the charged ink droplets just after attaching to the image-receiving layer can quickly lose their electric charge through earth. Thus, clear images free from disorder can be formed.

The specific electric resistance (also referred to as volume specific electric resistance or specific resistivity, sometimes) is measured by a three-terminal method with a guard electrode according to the method described in JIS K-6911.

The water-resistant support having the electric conductivity which can be preferably used will be described in more detail below.

The terms "electric conductivity" and "electrically conductive" are hereinafter abbreviated as "conductivity" and "conductive" respectively.

First, the support that is conductive as the whole is described below.

Such a support can be prepared by using as a substrate a conductive base paper, such as paper impregnated with sodium chloride, and providing a conductive water-resistant layer on both sides of the substrate. Examples of paper which can be used for preparing the conductive base paper include wood pulp paper, synthetic pulp paper, and paper made from a mixture of wood pulp and synthetic pulp. It is preferred for such paper to have a thickness of 80 to 200  $\mu\text{m}$ .

The formation of the conductive layer can be performed by applying a layer containing a conductive filler and a binder on the both sides of the conductive paper. The thickness of each of the conductive layer applied is preferably from 5 to 20  $\mu\text{m}$ .

Examples of the conductive filler usable include granular carbon black or graphite, metal powder such as silver, copper, nickel, brass, aluminum, steel or stainless steel powder, tin oxide powder, flaky aluminum or nickel, and fibrous carbon.

The binder can be appropriately selected from various kinds of resins. Examples of a resin suitable for the binder include hydrophobic resins, for example, acrylic resins, vinyl chloride resins, styrene resins, styrene-butadiene

resins, styrene-acrylic resins, urethane resins, vinylidene chloride resins and vinyl acetate resins, and hydrophilic resins, for example, polyvinyl alcohol resins, cellulose derivatives, starch and derivatives thereof, polyacrylamide resins and copolymers of styrene and maleic anhydride.

Another method for forming the conductive layer is to laminate a conductive thin film. Examples of such a conductive thin film usable include a metallic foil and a conductive plastic film. More specifically, an aluminum foil can be used for the metallic foil, and a polyethylene resin film in which carbon black is incorporated can be used for the conductive plastic film. Both hard and soft aluminum foils can be used as the laminating material. The thickness of the conductive thin films is preferably from 5 to 20  $\mu\text{m}$ .

For the lamination of a polyethylene resin in which carbon black is incorporated, it is preferred to adopt an extrusion lamination method. This method includes the steps of melting the polyethylene resin by heating, forming the molten resin into a film, pressing the film immediately against the base paper and the composite cooling, and can be carried out with various well-known apparatuses. The thickness of the laminated layer is preferably from 10 to 30  $\mu\text{m}$ . As the support having conductivity as a whole, a conductive plastic film and a metal plate can be used as they are as far as they have a satisfactory water-resistant property.

The conductive plastic film includes, e.g., a polypropylene or polyester film in which a conductive filler such as carbon fiber or carbon black is incorporated, and the metal plate includes, e.g., an aluminum plate. The thickness of a substrate is preferably from 80 to 200  $\mu\text{m}$ . When the substrate has a thickness of less than 80  $\mu\text{m}$ , it may not ensure sufficient strength in the printing plate. On the other hand, when the thickness of the substrate is more than 200  $\mu\text{m}$ , the handling property such as transportability in a recording apparatus may tend to decrease.

The support having a conductive layer provided on one side or both sides of the water-resistant substrate is described below.

As the water-resistant substrate, paper subjected to water-resistant treatment, paper laminated with a plastic film or a metal foil and a plastic film each preferably having a thickness of from 80 to 200  $\mu\text{m}$  can be used.

As a method for forming a conductive layer on the substrate, the same methods as described in the case where the whole of the support is conductive, can be used. More specifically, the composition containing a conductive filler and a binder is coated on one side of the substrate to form a layer having a thickness of from 5 to 20  $\mu\text{m}$ . Also, the conductive layer is formed by laminating a metal foil or a conductive plastic film on the substrate.

Another method which may be employed comprises depositing a metal film such as an aluminum, tin, palladium or gold film onto a plastic film.

Thus, the water-resistant support having the electrically conductive property can be obtained.

For preventing the printing plate precursor from curling, the support may have a backcoat layer (backing layer) on the side opposite to the image-receiving layer. It is preferred that the backcoat layer has the Bekk smoothness of 150 to 700 (sec/10 ml). By providing such a backcoat layer on the support, the printing plate obtained can be mounted exactly in an offset printing machine without suffering shear or slippage.

The thickness of the water-resistant support provided with the under layer and/or the backcoat layer is from 90 to 130  $\mu\text{m}$ , more preferably from 100 to 120  $\mu\text{m}$ .

Image formation on the lithographic printing plate precursor can be performed by any appropriate method, for

example, an electrophotographic recording system, an ink jet recording system or a thermal transfer recording system.

The electrophotographic recording system employed may be any of various well-known recording systems. For instance, the recording systems described, e.g., in Denshishashin Gakkai ed., *Denshishashin Gijutsu no Kiso to Oyo (The Fundamentals and Applications of Electrophotographic Techniques)*, Corona Co. (1988), Kenichi Eda, *Denshishashin Gakkai Shi (Journal of Electrophotographic Society)*, 27, 113 (1988), and Akio Kawamoto, *ibid.*, 33, 149 (1994) and Akio Kawamoto, *ibid.*, 32, 196 (1993); and commercially available PPC duplicating machines can be employed.

A combination of an exposure system in which the exposure is performed by scanning the laser beams based on digital information with a development system using a liquid developer can be adopted as an effective method for image formation, because it enables the formation of highly accurate images. One example utilizing such a combination is illustrated below.

A photosensitive material is positioned on a flat bed by a register pin system, and fixed to the flat bed by undergoing air suction from the back side. Then, the photosensitive material is charged by means of a charging device described, e.g., in the above-described reference, *The Fundamentals and Applications of Electrophotographic Techniques*, p. 212 et seq. Specifically, a corotron or scotron system is ordinarily used for charging. At the time of charging, it is also preferred to control the charging condition so that the surface potential of the photosensitive material is always kept within the intended range through a feedback system based on the information from a means of detecting the potential of the charged photosensitive material. Thereafter, the scanning exposure using a laser-beam source is performed according to, e.g., the method as described in the reference described above, p. 254 et seq.

Then, toner image formation is carried out with a liquid developer. The photosensitive material charged and exposed on the flat bed is detached from the flat bed, and subjected to wet development as described in the reference described above, p. 275 et seq. The exposure has been carried out in a mode corresponding to the toner image development mode. In the case of reversal development, for instance, a negative image, or an image area, is exposed to laser beams, a toner having the same charge polarity as the charged photosensitive material is employed, and the toner is adhered electrically to the exposed area by applying a bias voltage for development. The principle of this process is explained in detail in the reference described above, p. 157 et seq.

For removal of excess developer after development, the photosensitive material is squeegeed with a rubber roller, a gap roller or a reverse roller, or subjected to corona squeegee or air squeegee as described at page 283 of the above-described reference. Before such a squeegee treatment, the photosensitive material is preferably rinsed with only a carrier liquid of the liquid developer.

Then, the toner image formed on the photosensitive material is transferred onto the lithographic printing plate precursor according to the present invention directly or via a transfer intermediate, and fixed to the printing plate precursor.

Any of conventionally known ink jet recording systems can be employed for the image formation. However, the use of oil-based ink is desirable because it ensures quick drying and satisfactory fixation of the ink image and less clogging, and the adoption of an electrostatic ejection type ink jet

recording system is preferable, because such a system hardly causes blur of image. A solid jet type ink jet recording system using hot-melt ink is also preferably used.

For the electrostatic ejection type ink jet recording system, recording apparatus described in WO 93/11866, Wo 97/27058 and WO 97/27060 can be employed. The oil-based ink to be used is preferably a dispersion comprising hydrophobic resin particles, which are solid at least at normal temperature (i.e., 15 to 35° C.), dispersed in a nonaqueous solvent having an electric resistance of  $10^9 \Omega \cdot \text{cm}$  or more and a dielectric constant of 3.5 or below as a dispersion medium. By using such a nonaqueous solvent as the dispersion medium, the electric resistance of the oil-based ink is appropriately controlled and thus, the ejection of the oil-based ink by the action of an electric field can be properly carried out, whereby the image quality obtained is improved. Further, the use of the resin particles described above can provide enhanced affinity for the image-receiving layer and as a result, images of good quality are obtained as well as printing durability of the resulting printing plate is increased.

Specific examples of the oil-based ink suitable for use is described, for example in U.S. patent application Ser. No. 09/008,544, now U.S. Pat. No. 6,143,806, Ser. No. 09/085,100, now U.S. Pat. No. 6,174,936, Ser. No. 09/009,692, now U.S. Pat. No. 6,184,267, Ser. No. 09/009,131, now U.S. Pat. No. 6,197,847, Ser. No. 09/066,600, now U.S. Pat. No. 6,127,452, JP-A-10-204354 and JP-A-306244.

For the solid jet type ink jet recording system, commercially available printing systems such as Solid Inkjet Plate-maker SJ02A (manufactured by Hitachi Koki Co., Ltd.) and MP-1200Pro (manufactured by Dynic Co., Ltd.) are employed.

A method for forming an image on the lithographic printing plate precursor according to the present invention using an ink jet recording system is described in more detail with reference to FIG. 1 to FIG. 3 below.

A device system shown in FIG. 1 comprises an ink jet recording device 1 wherein oil-based ink is used.

As shown in FIG. 1, pattern information of images (figures and letters) to be formed on a lithographic printing plate precursor (also referred to as "master" hereinafter) 2 is first supplied from an information supply source such as a computer 3 to the ink jet recording device 1 using oil-based ink through a transmission means such as a bus 4. A head for ink jet recording 10 of the recording device 1 stores oil-based ink inside. When the master 2 is passed through the ink jet recording device 1, the head 10 ejects minute droplets of the ink onto the master 2 in accordance with the above described information, whereby the ink is attached to the master 2 in the above described pattern. Thus, the image formation on the master 2 is completed, whereby the lithographic printing plate precursor having the images thereon is obtained.

One example of the ink jet recording device as shown in the device system of FIG. 1 is depicted in FIG. 2 and FIG. 3, respectively. In FIG. 2 and FIG. 3, members common to the members in FIG. 1 are designated using the same symbols, respectively.

FIG. 2 is a schematic view showing the main part of the ink jet recording device, and FIG. 3 is a partially cross sectional view of the head.

As shown in FIG. 2 and FIG. 3, the head 10 installed in the ink jet recording device has a slit between an upper unit 101 and a lower unit 102, a leading edge thereof forms an ejection slit 10a. Further, an ejection electrode 10b is arranged in the slit, and the interior of the slit is filled with oil-based ink 11.

To the ejection electrode 10b of the head 10, a voltage is applied in accordance with digital signals from the pattern information of image. As shown in FIG. 2, a counter electrode 10c is arranged so as to face with the ejection electrode 10b, and the master 2 is provided on the counter electrode 10c. By the application of the voltage, a circuit is formed between the ejection electrode 10b and the counter electrode 10c, and the oil-based ink 11 is ejected from the ejection slit 10a of the head 10, thereby forming an image on the master 2 provided on the counter electrode 10c.

With respect to the width of the ejection electrode 10b, it is preferred for the leading edge thereof to be as narrow as possible in order to form an image of high quality.

For instance, print of  $40 \mu\text{m}$ -dot can be formed on the master 2 by filling the head 10 as shown in FIG. 3 with the oil-based ink, disposing the ejection electrode 10b having a leading edge having a width of  $20 \mu\text{m}$  and the counter electrode 10c so as to face with each other at a distance of 1.5 mm and applying a voltage of 3 KV for 0.1 millisecond between these two electrodes.

Another example of the ink jet recording device is depicted in FIG. 4 and FIG. 5.

FIG. 4 is a schematic view showing only the main part of a head for explanation. An ink jet recording head 13 comprises a body of head 14 made of an insulating material such as plastics, ceramics or glass, and meniscus regulation boards 15 and 16 as shown in FIG. 4. The symbol 17 in the figure stands for an ejection electrode to which a voltage is applied to form an electrostatic field at an ejection part.

The body of head is illustrated in more detail with reference to FIG. 5 wherein the regulation boards 15 and 16 are removed. The body of head 14 has plural ink grooves 18 cut perpendicularly to the edge thereof for the purpose of ink circulation. Each ink groove is designed to exert capillarity enough to form a uniform ink flow. Preferably, a width of the ink groove is from 10 to  $200 \mu\text{m}$ , and a depth thereof is from 10 to  $300 \mu\text{m}$ . The ejection electrodes 17 are provided in the grooves respectively. The ejection electrode is formed on the body of head 14 made of an insulating material using an conductive material such as aluminum, nickel, chromium, gold or platinum in a known manner. The ejection electrode may be formed on the entire inner surface or a part of the inner surface of the ink groove 18. Each ejection electrode is formed electrically independent.

Two ink grooves adjacent to each other form one cell, and a separator wall 19 is provided in the center of the cell. The separator wall has an ejection part 20 or 20' in its tip part. The separator wall is made thinner in the ejection part 20 or 20' than the other part thereof, and the ejection part is sharpened. The tip of the ejection part may be slightly cut off as shown by the ejection part 20'. The body of head can be produced by a known method such as machining or etching a block of an insulating material or molding an insulating material. The thickness of the ejection part of the separator wall is preferably from 5 to  $50 \mu\text{m}$ , and the sharpened ejection part preferably has a radius of curvature of from 5 to  $50 \mu\text{m}$ . While only two cells are depicted in the figure, between two cells, the separator wall 21 is disposed, and the tip part thereof 22 is cut off so as to stand back compared with the ejection parts 20 and 20'.

The ink is flowed into the head via the ink grooves from the direction represented by the arrow I by means of an ink supplying device (not shown) to supply the ink to the ejection parts. The excess ink is recovered in the direction represented by the arrow O by means of a recovering device (not shown). As a result, fresh ink is always supplied to each ejection part. A counter electrode holding a lithographic

printing plate precursor on its surface (not shown) is arranged so as to face the ejection part. The ink around the ejection part is irradiated with light as shown by the arrow L. While keeping such a condition, a signal voltage corresponding to the image data is applied to the ejection electrode, and the ink is ejected from the ejection part to form an image on the lithographic printing plate precursor.

The lithographic printing plate precursor having the image formed thereon by the ink jet recording system using the oil-based ink as described above can be used as it is as a lithographic printing plate.

According to the use of the direct drawing type lithographic printing plate precursor of the present invention, images free from not only background stain over an entire surface but also dot-like stain can be formed thereon. Also, the direct drawing type lithographic printing plate precursor can prepare a lithographic printing plate providing a great number of printed matter having clear images free from disappearance or distortion of image.

The present invention will be described in greater detail with reference to the following examples, but the present invention should not be construed as being limited thereto.

#### EXAMPLE 1

A mixture of 100 g of zinc oxide (Finex-50 manufactured by Sakai Chemical Industry Co., Ltd.; average particle size: 40 nm), 113 g of a 10% by weight aqueous solution of polyvinyl alcohol (PVA 117 manufactured by Kuraray Co., Ltd.) and 240 g of water was dispersed together with glass beads in a paint shaker (manufactured by Toyo Seiki Seisakusho Corp.) for 30 minutes. Then, to the dispersion were added 110 g of a 20% by weight water/ethanol (1:1 in a weight ratio) solution of tetraethoxysilane hydrolyzed previously and 200 g of a 20% by weight aqueous dispersion of colloidal silica (Snowtex C manufactured by Nissan Chemical Industries, Ltd.) and the mixture was dispersed for 3 minutes, followed by removing the glass beads to prepare a coating composition for image-receiving layer.

A support for ELP-2X Type Master (manufactured by Fuji Photo Film Co., Ltd.) having the Bekk smoothness of 2,000 (sec/10 ml) on the under layer side, which is used as an electrophotographic lithographic printing plate precursor for small-scale commercial printing, was employed. On the support, the coating composition for image-receiving layer prepared above was coated by means of a wire bar and dried in an oven at 100° C. for 10 minutes to form an image-receiving layer having a coating amount of 8 g/m<sup>2</sup>. Thus, a lithographic printing plate precursor was prepared.

#### Comparative Example 1A

A lithographic printing plate precursor was prepared in the same manner as in Example 1 except for using 100 g of titanium oxide (TiO<sub>2</sub>, average particle size: 0.3 μm) in place of 100 g of zinc oxide (Finex-50).

The lithographic printing plate precursors prepared in Example 1 and Comparative Example 1A were subjected to evaluating their properties, respectively. The results obtained are shown in Table A-1 below.

TABLE A-1

|    | Example 1                                                             | Comparative Example 1A                                                                                                           |                                                                                                                                    |
|----|-----------------------------------------------------------------------|----------------------------------------------------------------------------------------------------------------------------------|------------------------------------------------------------------------------------------------------------------------------------|
| 5  | Surface Smoothness of Image-receiving Layer <sup>1)</sup> (sec/10 ml) | 300                                                                                                                              | 255                                                                                                                                |
| 10 | Contact Angle with Water <sup>2)</sup> (degree)                       | 0                                                                                                                                | 0                                                                                                                                  |
| 15 | Image Reproducibility <sup>3)</sup>                                   | neither blur nor distortion of fine lines and fine letters; shape of dot: true circle; sufficient density in solid image portion | neither blur nor distortion of fine lines and fine letters; shape of dot: true circle; insufficient density in solid image portion |
| 20 | Press Life <sup>4)</sup>                                              | 10,000 sheets                                                                                                                    | 1,500 sheets                                                                                                                       |

The properties described in Table A-1 were evaluated in the following manner.

#### Surface Smoothness of Image-receiving Layer<sup>1)</sup>

A Bekk smoothness of the surface of the lithographic printing plate precursor was measured using a Bekk smoothness tester (manufactured by Kumagai Riko Co., Ltd.) under the condition of the air volume of 10 ml.

#### Contact Angle with Water<sup>2)</sup>

On the surface of the lithographic printing plate precursor was put 2 μl of distilled water, and after a 30-second lapse at room temperature a contact angle of the lithographic printing plate precursor surface with water was measured using a surface contact angle meter (CA-D manufactured by Kyowa Kaimen Kagaku Co., Ltd.).

#### Image Reproducibility<sup>3)</sup>

A servo plotter (DA 8400 manufactured by Graphtech Co.) able to write in accordance with an output from a personal computer was converted so that an ink ejection head as shown in FIG. 4 was mounted on a pen plotter section, and the lithographic printing plate precursor described above was placed on a counter electrode positioned at a distance of 500 μm from the ink ejection head. Ink jet printing was performed on the lithographic printing plate precursor using Oil-Based Ink (IK-1) shown below to conduct image formation. Then, the printing plate precursor was heated by means of a Ricoh Fuser (Model 592 manufactured by Ricoh Co., Ltd.) so as to control the surface temperature of the printing plate precursor to 80° C. for one minute, thereby thoroughly fixing the ink image.

50 The image formed on the printing plate precursor was visually observed under an optical microscope of 200 magnifications.

#### <Preparation of Oil-Based Ink (IK-1)>

A mixed solution of 12 g of Dispersion Stabilizing Resin (PS-1) shown below, 100 g of vinyl acetate and 321 g of Isopar G was heated to a temperature of 75° C. under nitrogen gas stream with stirring. To the solution was added 1.5 g of 2,2'-azobis(isovaleronitrile) (abbreviated as AIVN) as a polymerization initiator, followed by reacting for 3 hours. Further, 1.0 g of AIVN was added to the reaction mixture, followed by reacting for 3 hours. Then, the temperature of the reaction mixture was raised to 100° C., followed by stirring for 2 hours, thereby distilling off the unreacted vinyl acetate. After cooling the reaction mixture, it was passed through a nylon cloth of 200 mesh. The resulting white dispersion was a latex of good monodispersity having a polymerization rate of 93% and an average

particle size of  $0.38 \mu\text{m}$ . The particle size was measured by CAPA-500 manufactured by Horiba Ltd.  
Dispersion Stabilizing Resin (PS-1)



Mw:  $4 \times 10^4$

A part of the above-described white dispersion was centrifuged at a rotation of  $1 \times 10^4$  r.p.m. for 60 minutes and the resin particles precipitated were collected and dried. A weight average molecular weight (Mw) of the resin particles was measured by a GPC method and calculated in terms of polystyrene. The weight average molecular weight (Mw) of the resin particles was  $2 \times 10^5$ , and a glass transition point (Tg) thereof was  $38^\circ\text{C}$ . The resulting resin particle was designated as Resin Particle (PL-1).

Ten grams of dodecyl methacrylate/acrylic acid copolymer (copolymerization ratio: 95/5 by weight), 10 g of nigrosine and 30 g of Isopar G were placed in a paint shaker (manufactured by Toyo Seiki Seisakusho Corp.) together with glass beads and dispersed for 4 hours to obtain a fine dispersion of nigrosine.

Sixty grams (as a solid basis) of Resin Particle (PL-1) described above, 7.5 g of the above-described nigrosine dispersion and 0.06 g of dodecene-maleic acid mono-octadecylamide copolymer were diluted with one liter of Isopar E, thereby obtaining black-colored Oil-Based Ink (IK-1). Press Life<sup>4)</sup>

The image formation on the lithographic printing plate precursor and fixing of the image were conducted in the same manner as described in the image reproducibility<sup>3)</sup> above to prepare a lithographic printing plate.

The lithographic printing plate thus prepared was subjected to printing using as a printing machine, Oliver Model 4094 manufactured by Sakurai Seisakusho Co., Ltd., as dampening water, a solution prepared by diluting EU-3 (manufactured by Fuji Photo Film Co., Ltd.) 50 times with water and black ink for offset printing.

A number of printed matter obtained without background stain and disappearance of fine lines and fine letters was determined as the press life.

As shown in Table A-1 above, the surface smoothness of the image-receiving layer was almost same in Example 1 and Comparative Example 1A. The contact angle with water was 0 degree in each example. This means that the surface has good hydrophilicity. With respect to the printing plate formed by plate-making in Example 1, neither blur nor distortion of fine lines and fine letters were observed, the density in the solid image portion was sufficiently high, and the dot image had true circular shape. On the contrary, the printing plate formed by plate-making in Comparative Example 1A had insufficient density in the solid image portion, although the reproducibility of fine lines and fine letters and the shape of dot were same as those in Example 1.

As a result of the printing, 10,000 sheets of printed matter having clear images free from stain due to adhesion of printing ink were obtained in Example 1. In Comparative Example 1A, on the contrary, disappearance of the image area occurred after printing about 1,500 sheets, while stain in the non-image area was not observed.

Each lithographic printing plate precursor was prepared in the same manner as in Example 1 except for using 100 g of each of the compounds (the average particle size of each compound being in a range of from  $0.03$  to  $2 \mu\text{m}$ ) shown in Table B-1 below in place of 100 g of zinc oxide (Finex-50).

With each of the lithographic printing plate precursors, the Belkk smoothness of the surface thereof was in a range of from 250 to 300 (sec/10 ml), and the contact angle of the surface thereof with water was 0 degree.

Each lithographic printing plate precursor was subjected to plate-making and printing in the same manner as in Example 1. The printed matter obtained had clear images free from background stain in the non-image area and blur and distortion of fine lines and fine letters. The press life of each lithographic printing plate was good as more than 5,000 sheets as shown in Table B-1 below.

TABLE B-1

| Example | Metal Oxide          | Press Life |
|---------|----------------------|------------|
| 2       | Magnesium oxide      | 5,000      |
| 3       | Barium oxide         | 5,000      |
| 4       | Chromium (III) oxide | 8,000      |
| 5       | Cobalt (III) oxide   | 8,000      |
| 6       | Zirconium oxide      | 10,000     |
| 7       | Stannic oxide        | 8,000      |
| 8       | Nickel oxide         | 10,000     |
| 9       | Molybdenum trioxide  | 8,000      |
| 10      | Tungsten dioxide     | 10,000     |
| 11      | Tungsten trioxide    | 10,000     |
| 12      | Cuprous oxide        | 10,000     |
| 13      | Lead (IV) oxide      | 9,000      |
| 14      | Trilead tetroxide    | 9,000      |
| 15      | Vanadium (IV) oxide  | 8,000      |
| 16      | Manganese (II) oxide | 8,000      |
| 17      | Lanthanum oxide      | 6,000      |
| 18      | Germanium (IV) oxide | 5,000      |

## EXAMPLE 19

60 <Preparation of Direct Drawing Type Lithographic Printing Plate Precursor>

A composition having the following component was placed in a paint shaker (manufactured by Toyo Seiki Seisakusho Corp.) together with glass beads and dispersed for 30 minutes at room temperature. Then, the glass beads were removed by filtration to obtain a dispersion.

|                                                                                                                   |       |
|-------------------------------------------------------------------------------------------------------------------|-------|
| Cobalt (II) oxide (average particle size: 1.7 $\mu\text{m}$ )                                                     | 45 g  |
| 10% By weight aqueous solution of gelatin                                                                         | 100 g |
| 20% By weight aqueous dispersion of colloidal silica (Snowtex C manufactured by Nissan Chemical Industries, Ltd.) | 25 g  |
| Tetraethoxysilane                                                                                                 | 30 g  |
| Fluorinated alkyl ester (FC-430 manufactured by 3M Co.)                                                           | 0.2 g |
| Hardening agent                                                                                                   | 0.5 g |
| $\text{CH}_2=\text{CHSO}_2\text{CH}_2\text{CONH}(\text{CH}_2)_3\text{NHCOCH}_2\text{SO}_2\text{CH}=\text{CH}_2$   |       |
| 1N Hydrochloric acid                                                                                              | 2 g   |
| Solvent mixture of water and ethanol (1/1 in weight ratio)                                                        | 200 g |

On a support for ELP-2X Type Master, the coating composition prepared above was coated by means of a wire bar, set to touch and then heated at 110° C. for 30 minutes to form an image-receiving layer having a coating amount of 6 g/m<sup>2</sup>. Thus, a lithographic printing plate precursor was prepared.

The Bekk smoothness of the surface of the lithographic printing plate precursor was 450 (sec/10 ml), and the contact angle of the surface with water was 0 degree.

**<Preparation of Electrophotographic Light-Sensitive Element>**

A mixture of 2 g of X-type metal-free phthalocyanine (manufactured by Dai-Nippon Ink & Chemicals Inc.), 14.4 g of Binder Resin (P-1) shown below, 3.6 g of Binder Resin (P-2) shown below, 0.15 g of Compound (A) shown below and 80 g of cyclohexanone was placed together with glass beads in a 500 ml of glass vessel, and dispersed for 60 minutes by a paint shaker (manufactured by Toyo Seiki Seisakusho Corp.). Then, the glass beads was removed by filtration to prepare a dispersion for light-sensitive layer.

**Binder Resin (P-1)**



Mw:  $6 \times 10^4$

**Binder Resin (P-2)**



Mw:  $8 \times 10^3$

**Compound (A)**



The dispersion thus prepared was coated on a 0.2 mm-thick degreased aluminum plate by means of a wire bar,

set to touch, and then heated for 20 seconds in a circulation type oven regulated at 110° C. The thus-formed light-sensitive layer had a thickness of 8  $\mu\text{m}$ .

The electrophotographic light-sensitive element prepared above was subjected to corona discharge in the dark to gain the surface potential of +450 V, and then to scanning-exposure by a semiconductor laser drawing device with a beam of 788 nm as an exposure apparatus. The laser beam scanning was performed on the basis of image information which was obtained by previously reading an original with a color scanner, subjecting the read image information to color separation, making some corrections relating to color reproduction of the system used, and then memorizing the corrected image information as digital image data in the internal hard disk of the system. As to the laser beam scanning condition, the beam spot diameter was 15  $\mu\text{m}$ , the pitch was 10  $\mu\text{m}$  and the scanning speed was 300 cm/sec (i.e., 2,500 dpi). The amount of exposure on the light-sensitive element was adjusted to 25 erg/cm<sup>2</sup>.

Subsequently, the light-sensitive element exposed in the manner described above was developed with a liquid developer shown below, rinsed in a bath of Isopar G alone to remove stain in the non-image area, and dried with a hot air so that the light-sensitive element had a surface temperature of 50° C. and the amount of residual Isopar G was reduced to 10 mg per g of the toner. Then, the light-sensitive element was subjected to -6 kV precharge with a corona charging device, and the image side of the light-sensitive element was brought into face-to-face contact with the lithographic printing plate precursor described above and underwent negative corona discharge on the side of the light-sensitive element, thereby performing the image transfer.

**<Preparation of Liquid Developer>**

The following ingredients were mixed and kneaded for 2 hours at 95° C. by means of a kneader to prepare a mixture. The mixture was cooled inside the kneader, and then ground to powder therein. The powder in an amount of 1 parts by weight and Isopar H in an amount of 4 parts by weight were dispersed for 6 hours by a paint shaker to prepare a dispersion. The resulting dispersion was diluted with Isopar G so as to have a solid toner content of 1 g per liter and, as a charge control agent for imparting a negative charge, basic barium petronate was added thereto in an amount of 0.1 g per liter. Thus, a liquid developer was prepared.

**Ingredients to Be Kneaded**

|                                                                                       |                    |
|---------------------------------------------------------------------------------------|--------------------|
| Ethylene-methacrylic acid copolymer (Nucrel N-699 manufactured by Mitsui Du Pont Co.) | 4 parts by weight  |
| Carbon Black #30 (manufactured by Mitsubishi Chemical Industries Ltd.)                | 1 parts by weight  |
| Isopar L (manufactured by Exxon Corp.)                                                | 15 parts by weight |

The lithographic printing plate precursor having the image formed thereon was heated at 100° C. for 30 seconds, thereby fixing completely the toner image.

The image formed on the lithographic printing plate precursor was observed under an optical microscope of 200 magnifications to evaluate its image quality. The image formed was clear and free from blur and disappearance of fine lines and fine letters.

Then, the lithographic printing plate thus-prepared was mounted in a printing machine (Oliver Model 94 manufactured by Sakurai Seisakusho Co., Ltd.), and printing was performed on sheets of printing paper using black ink for

offset printing and dampening water prepared by diluting SLM-OD (manufactured by Mitsubishi Paper Mills, Ltd.) 100 times with distilled water and supplied in a dampening saucer.

The 10th printed matter was picked up in the course of printing, and the printed image thereon was evaluated by visual observation using a magnifier of 20 magnifications. The observation result indicated that the non-image area was free from background stain due to adhesion of the printing ink and the uniformity of the solid image portion was good. Further, the printed matter was observed under an optical microscope of 200 magnifications. According to the observation, neither sharpening nor disappearance were found in the area of fine lines and fine letters, and the image quality of printed matter was good.

As a result of continuing the printing procedure, more than 10,000 sheets of printed matter having image quality equal to that of the 10th print were obtained.

#### EXAMPLE 20

##### <Preparation of Water-Resistant Support>

Water-resistant base paper having a basis weight of 100 g/m<sup>2</sup> and a thickness of 115 µm was used as a substrate, and polyethylene was laminated on both surfaces of the paper to prepare water-proof paper having the polyethylene layer of 15 µm on one side and the polyethylene layer of 20 µm on the other side.

A coating composition for under layer shown below was coated on the polyethylene layer of 15 µm by means of a wire bar to form an under layer having a dry coating amount of 10 g/m<sup>2</sup>. Then, the under layer was subjected to a calender treatment so as to have the Bekk smoothness of about 1,500 (sec/10 ml).

##### Coating Composition for Under Layer

The following composition was mixed and water was added thereto so as to have a total solid concentration of 25% to prepare the coating composition for under layer.

|                                                           |            |
|-----------------------------------------------------------|------------|
| Carbon black (30% aqueous dispersion)                     | 7.2 parts  |
| Clay (50% aqueous dispersion)                             | 52.8 parts |
| SBR latex (solid content: 50%, Tg: 25° C.)                | 36 parts   |
| Melamine resin (solid content: 80%, Sumirez Resin SR-613) | 4 parts    |

The measurement of specific electric resistance of the under layer was carried out in the following manner.

The coating composition for under layer was applied to a thoroughly degreased and cleaned stainless steel plate at a dry coating amount of 10 g/m<sup>2</sup> to form a coating film. The thus formed coating film was examined for specific electric resistance in accordance with a three-terminal method with a guard electrode according to the method described in JIS K-6911. The value obtained was 1×10<sup>8</sup> Ω.cm.

##### <Preparation of Direct Drawing Type Lithographic Printing Plate Precursor>

A composition for image-receiving layer having the following component was placed in a paint shaker (manufactured by Toyo Seiki Seisakusho Corp.) together with glass beads and dispersed for 20 minutes at room temperature. Then, the glass beads were removed by filtration to obtain a dispersion.

|                                                                                                        |       |
|--------------------------------------------------------------------------------------------------------|-------|
| Manganese dioxide (average particle size: 1.5 µm)                                                      | 80 g  |
| 10% By weight aqueous solution of starch (Penon ZP-2 manufactured by Nichiden Chemical Co., Ltd.)      | 300 g |
| Clay                                                                                                   | 10 g  |
| Tetrapropoxysilane                                                                                     | 40 g  |
| Methyltrimethoxysilane                                                                                 | 3 g   |
| Alumina sol (520 manufactured by Nissan Chemical Industries, Ltd.; average particle size: 10 to 20 nm) | 10 g  |
| Ethanol                                                                                                | 110 g |
| 1N Hydrochloric acid                                                                                   | 5 g   |
| Water                                                                                                  | 150 g |

15

The dispersion was coated on the water-resistant support described above by means of a wire bar and dried in an oven at 100° C. for 20 minutes to form an image-receiving layer having a coating amount of 6 g/m<sup>2</sup>. Thus, a lithographic printing plate precursor was prepared.

The Bekk smoothness of the surface of the lithographic printing plate precursor was 150 (sec/10 ml), and the contact angle of the surface with water was 0 degree.

The lithographic printing plate precursor was subjected to plate-making by means of a laser printer (AM-SIS 1200-J Plate Setter) with dry toner commercially available as AM-Straight Imaging System.

The quality of duplicated image on the printing plate precursor thus obtained was visually evaluated through a magnifier of 20 magnifications, and it was found that the image quality was good. Specifically, the plate-making image formed by transfer of dry toner from the laser printer had no disappearance of fine lines and fine letters and uniform solid image portion, and unevenness of toner transfer was not observed at all. Although, the background stain due to scattering of toner was slightly occurred in the non-image area, it was practically acceptable.

The lithographic printing plate precursor was subjected to plate-making in the same manner as described above. The lithographic printing plate thus prepared was then subjected to printing using a full-automatic printing machine (AM-2850 manufactured by AM Co., Ltd.), a solution prepared by diluting a PS plate processing agent (EU-3 manufactured by Fuji Photo Film Co., Ltd.) 50 times with distilled water and supplied in a dampening saucer as dampening water, and black ink for offset printing. The 10th sheet was picked up in the course of printing, and the printed image thereon was visually evaluated for its image quality (background stain and uniformity in solid image portion) through a magnifier of 20 magnifications. The image quality was excellent.

As a result of continuing the printing procedure, 10,000 sheets of printed matter having image quality equal to that of the 10th print were obtained.

#### EXAMPLES 21 TO 27

Lithographic printing plate precursors were prepared in the same manner as in Example 1 except for using the organic polymer and the silane compound shown in Table C-1 below in place of polyvinyl alcohol (PVA 117) and thoxysilane, respectively.

TABLE C-1

| Example | Organic Polymer                                                                         | Silane Compound (weight ratio)                                                    |
|---------|-----------------------------------------------------------------------------------------|-----------------------------------------------------------------------------------|
| 21      | Polyvinylpyrrolidone                                                                    | Triethoxysilane (20%)<br>Tetramethoxysilane (80%)                                 |
| 22      | Propyleneoxide-modified starch (PENON HV-2 manufactured by Nichiden Chemical Co., Ltd.) | Tetra(2-methoxyethoxy)titanium (5%)<br>Tetrabutoxysilane (95%)                    |
| 23      | Hydroxypropylated starch (PENON LD-1 manufactured by Nichiden Chemical Co., Ltd.)       | Octyltrimethoxysilane (1%)<br>Tetrapropoxysilane (99%)                            |
| 24      | N-Methylolacrylamide/methyl acrylate (85/15 in weight ratio) copolymer                  | 3-Hydroxypropyltrimethoxysilane (5%)                                              |
| 25      | Polyethylene glycol 20,000 (manufactured by Wako Pure Chemical Industries, Ltd.)        | Tetraethoxysilane (95%)<br>Methyltrimethoxysilane (2%)<br>Tetraethoxysilane (98%) |
| 26      | Polyvinyl alcohol (PVA 405 manufactured by Kuraray Co., Ltd.)                           | 2-Carboxyethyltrimethoxysilane (5%)<br>Tetraethoxysilane (95%)                    |
| 27      |                                                                                         | Tetraethoxysilane (90%)<br>3-Sulfopropyltrimethoxysilane (10%)                    |

25

With each of the lithographic printing plate precursors, the Bekk smoothness of the surface thereof was in a range of from 250 to 300 (sec/10 ml), and the contact angle of the surface thereof with water was 0 degree.

Each of the lithographic printing plate precursor was subjected to plate-making and printing in the same manner as in Example 1. The printed matter obtained had clear images free from background stain in the non-image area similar to that obtained in Example 1. The press life of each lithographic printing plate was good, providing more than 10,000 sheets.

#### EXAMPLE 28

A composition having the following component was dispersed for 20 minutes using a paint shaker and coated on a support for ELP-2X Type Master by means of a wire bar, set to touch and then heated at 100° C. for 30 minutes to form an image-receiving layer having a coating amount of 6 g/m<sup>2</sup>. Thus, a lithographic printing plate precursor was prepared.

#### Composition for Image-receiving Layer

|                                                                                      |       |
|--------------------------------------------------------------------------------------|-------|
| Zinc oxide (Finex-50)                                                                | 45 g  |
| Silica (Silijsia 310 manufactured by Fuji Silijsia Chemical Co., Ltd.)               | 5 g   |
| Succinic acid-modified starch (PENON F3 manufactured by Nichiden Chemical Co., Ltd.) | 30 g  |
| Tetraethoxysilane                                                                    | 28 g  |
| Benzyltrimethoxysilane                                                               | 2 g   |
| 1N Hydrochloric acid                                                                 | 2 g   |
| Water                                                                                | 300 g |

The Bekk smoothness of the surface of the lithographic printing plate precursor was 300 (sec/10 ml), and the contact angle of the surface with water was not more than 5 degrees.

The lithographic printing plate precursor was subjected to plate-making using an electrostatic ejection type ink jet recording device as described in WO 93/11866 and Oil-Based Ink (IK-1) described in Example 1. The image formed on the lithographic printing plate precursor was clear and

free from distortion and blur in the accurate image portion such as fine lines and fine letters.

Using the printing plate thus obtained, printing was conducted in the same manner as in Example 1. The printed matter obtained had clear images free from background stain in the non-image area similar to that obtained in Example 1. The press life of the lithographic printing plate was good providing more than 10,000 sheets.

#### EXAMPLE 101

A lithographic printing plate precursor was prepared in the same manner as in Example 1 except for using 100 g of titanium hydroxide (Ti(OH)<sub>4</sub>, average particle size: 0.3 μm) in place of 100 g of zinc oxide (Finex-50).

#### Comparative Example 101A

A lithographic printing plate precursor was prepared in the same manner as in Example 101 except for using 100 g of titanium oxide (TiO<sub>2</sub>, average particle size: 0.3 μm) in place of 100 g of titanium hydroxide.

The lithographic printing plate precursors prepared in Example 101 and Comparative Example 101A were subjected to evaluating their properties in the same manner as described in Example 1, respectively. The results obtained are shown in Table A-101 below.

TABLE A-101

|                                                         | Example 101                                                 | Comparative Example 101A                                             |
|---------------------------------------------------------|-------------------------------------------------------------|----------------------------------------------------------------------|
| Surface Smoothness of Image-receiving Layer (sec/10 ml) | 280                                                         | 250                                                                  |
| Contact Angle with Water (degree)                       | 0                                                           | 0                                                                    |
| Image Reproducibility                                   | neither blur nor distortion of fine lines and fine letters; | neither blur nor distortion of fine lines and fine letters; shape of |

TABLE A-101-continued

|            | Example 101                                                                           | Comparative Example 101A                                                      |   |
|------------|---------------------------------------------------------------------------------------|-------------------------------------------------------------------------------|---|
| Press Life | shape of dot: true circle; sufficient density in solid image portion<br>10,000 sheets | dot: true circle; insufficient density in solid image portion<br>1,500 sheets | 5 |

As shown in Table A-101 above, the surface smoothness of the image-receiving layer was almost same in Example 101 and Comparative Example 101A. The contact angle with water was 0 degree in each example. This means that the surface has good hydrophilicity. With respect to the printing plate formed by plate-making in Example 101, neither blur nor distortion of fine lines and fine letters were observed, the density in the solid image portion was sufficiently high, and the dot image had true circular shape. On the contrary, the printing plate formed by plate-making in Comparative Example 101A had insufficient density in the solid image portion, although the reproducibility of fine lines and fine letters and the shape of dot were same as those in Example 101.

As a result of the printing, 10,000 sheets of printed matter having clear images free from stain due to adhesion of printing ink were obtained in Example 101. In Comparative Example 101A, on the contrary, disappearance of the image area occurred after printing about 1,500 sheets, while stain in the non-image area was not observed.

## EXAMPLES 102 TO 111

Each lithographic printing plate precursor was prepared in the same manner as in Example 101

except for using 100 g of each of the compounds (the average particle size of each compound being in a range of from 0.03 to 2  $\mu\text{m}$ ) shown in Table B-101 below in place of 100 g of titanium hydroxide.

With each of the lithographic printing plate precursors, the Bekk smoothness of the surface thereof was in a range of from 250 to 300 (sec/10 ml), and the contact angle of the surface thereof with water was 0 degree.

Each lithographic printing plate precursor was subjected to plate-making in the same manner as in Example 101. The printing plate precursor subjected to the plate-making had clear images free from disappearance, blur and distortion of fine lines and fine letters. The lithographic printing plate thus-prepared was subjected to printing in the same manner as in Example 101. The press life of each lithographic printing plate was good as more than 3,000 sheets as shown in Table B-101 below.

TABLE B-1

| Example | Metal Hydroxide     | Press Life |
|---------|---------------------|------------|
| 102     | Magnesium hydroxide | 3,000      |
| 103     | Barium hydroxide    | 4,000      |
| 104     | Aluminum hydroxide  | 6,000      |

TABLE B-1-continued

| Example | Metal Hydroxide       | Press Life |
|---------|-----------------------|------------|
| 105     | Zinc hydroxide        | 10,000     |
| 106     | Cobalt (II) hydroxide | 9,000      |
| 107     | Cupric hydroxide      | 8,000      |
| 108     | Nickel hydroxide      | 10,000     |
| 109     | Germanium hydroxide   | 10,000     |
| 110     | Tin hydroxide         | 8,000      |
| 111     | Lanthanum hydroxide   | 6,000      |

## EXAMPLE 112

<Preparation of Direct Drawing Type Lithographic Printing Plate Precursor>

A composition having the following component was placed in a paint shaker (manufactured by Toyo Seiki Seisakusho Corp.) together with glass beads and dispersed for 30 minutes at room temperature. Then, the glass beads were removed by filtration to obtain a dispersion.

|                                                                                                                   |        |
|-------------------------------------------------------------------------------------------------------------------|--------|
| Nickel hydroxide (manufactured by Nakarai Co., Ltd; average particle size: 40 nm)                                 | 42.5 g |
| 10% By weight aqueous solution of gelatin                                                                         | 100 g  |
| 20% By weight aqueous dispersion of colloidal silica (Snowtex C manufactured by Nissan Chemical Industries, Ltd.) | 37 g   |
| Tetraethoxysilane                                                                                                 | 15 g   |
| Fluorinated alkyl ester (FC-430 manufactured by 3M Co.)                                                           | 0.2 g  |
| Hardening agent                                                                                                   | 0.5 g  |
| $\text{CH}_2=\text{CHSO}_2\text{CH}_2\text{CONH}(\text{CH}_2)_3\text{NHCOCH}_2\text{SO}_2\text{CH}=\text{CH}_2$   |        |
| 1N Hydrochloric acid                                                                                              | 2 g    |
| Solvent mixture of water and ethanol (1/1 in weight ratio)                                                        | 200 g  |

On a support for ELP-2X Type Master, the coating composition prepared above was coated by means of a wire bar, set to touch and then heated at 110° C. for 30 minutes to form an image-receiving layer having a coating amount of 6 g/m<sup>2</sup>. Thus, a lithographic printing plate precursor was prepared.

The Bekk smoothness of the surface of the lithographic printing plate precursor was 800 (sec/10 ml), and the contact angle of the surface with water was not more than 5 degrees.

The lithographic printing plate precursor was subjected to plate-making in the same manner as in Example 19.

The image formed on the lithographic printing plate precursor was observed under an optical microscope of 200 magnifications to evaluate its image quality. The image formed was clear and free from blur and disappearance of fine lines and fine letters.

Then, the lithographic printing plate thus-prepared was subjected to printing in the same manner as in Example 19.

The 10th printed matter was picked up in the course of printing, and the printed image thereon was evaluated by visual observation using a magnifier of 20 magnifications.

35

The observation result indicated that the non-image area was free from background stain due to adhesion of the printing ink and the uniformity of the solid image portion was good. Further, the printed matter was observed under an optical microscope of 200 magnifications. According to the observation, neither sharpening nor disappearance were found in the area of fine lines and fine letters, and the image quality of printed matter was good.

As a result of continuing the printing procedure, more than 10,000 sheets of printed matter having image quality equal to that of the 10th print were obtained.

## EXAMPLE 113

A lithographic printing plate precursor was prepared in the same manner as in Example 20 except for using a composition for image-receiving layer having the following component in place of the composition for image-receiving layer used in Example 20.

|                                                                                                        |       |
|--------------------------------------------------------------------------------------------------------|-------|
| Zinc hydroxide (average particle size: 0.5 $\mu\text{m}$ )                                             | 80 g  |
| 10% By weight aqueous solution of starch (Penon ZP-2 manufactured by Nichiden Chemical Co., Ltd.)      | 300 g |
| Clay                                                                                                   | 10 g  |
| Tetraethoxysilane                                                                                      | 30 g  |
| Methyltrimethoxysilane                                                                                 | 3 g   |
| Alumina sol (520 manufactured by Nissan Chemical Industries, Ltd.; average particle size: 10 to 20 nm) | 10 g  |
| Ethanol                                                                                                | 110 g |
| 1N Hydrochloric acid                                                                                   | 5 g   |
| Water                                                                                                  | 150 g |

The Bekk smoothness of the surface of the lithographic printing plate precursor was 150 (sec/10 ml), and the contact angle of the surface with water was 0 degree.

The lithographic printing plate precursor was subjected to plate-making in the same manner as in Example 20.

36

magnifier of 20 magnifications, and it was found that the image quality was good. Specifically, the plate-making image formed by transfer of dry toner from the laser printer had no disappearance of fine lines and fine letters and uniform solid image portion, and unevenness of toner transfer was not observed at all. Although, the background stain due to scattering of toner was slightly occurred in the non-image area, it was practically acceptable.

The lithographic printing plate precursor was subjected to plate-making in the same manner as described above. The lithographic printing plate thus prepared was then subjected to printing in the same manner as in Example 20. The 10th sheet was picked up in the course of printing, and the printed image thereon was visually evaluated for its image quality (background stain and uniformity in solid image portion) through a magnifier of 20 magnifications. The image quality was excellent.

As a result of continuing the printing procedure, 10,000 sheets of printed matter having image quality equal to that of the 10th print were obtained.

## EXAMPLE 114 TO 120

Lithographic printing plate precursors were prepared in the same manner as in Example 101 except for using the organic polymer and the silane compound shown in Table C-101 below in place of polyvinyl alcohol (PVA 117) and tetraethoxysilane, respectively.

TABLE C-101

| Example | Organic Polymer                                                                                                                 | Silane Compound (weight ratio)                                                    |
|---------|---------------------------------------------------------------------------------------------------------------------------------|-----------------------------------------------------------------------------------|
| 114     | Polyvinylpyrrolidone                                                                                                            | Triethoxysilane (20%)<br>Tetramethoxysilane (80%)                                 |
| 115     | Propyleneoxide-modified starch (PENON HV-2 manufactured by Nichiden Chemical Co., Ltd.)                                         | Tetra(2-methoxyethoxy)titanium (5%)                                               |
| 116     | Hydroxypropylated starch (PENON LD-1 manufactured by Nichiden Chemical Co., Ltd.)                                               | Tetrabutoxysilane (95%)<br>Octyltrimethoxysilane (1%)<br>Tetrapropoxysilane (99%) |
| 117     | N-Nethylolacrylamide/methyl acrylate (85/15 in weight ratio) copolymer                                                          | 3-Hydroxypropyltrimethoxysilane (5%)                                              |
| 118     | Polyethylene glycol 20,000 (manufactured by Wako Pure Chemical Industries, Ltd.)                                                | Tetraethoxysilane (95%)<br>Methyltrimethoxysilane (2%)<br>Tetraethoxysilane (98%) |
| 119     | Polyvinyl alcohol (PVA 405 manufactured by Kuraray Co., Ltd.)                                                                   | 2-Carboxyethyltrimethoxysilane (5%)<br>Tetraethoxysilane (95%)                    |
| 120     | $\text{---}(\text{N}(\text{COCH}_3)\text{---CH}_2\text{CH}_2)_{90}(\text{N}(\text{H})\text{---CH}_2\text{CH}_2)_{10}\text{---}$ | Tetraethoxysilane (90%)<br>3-Sulfopropyltrimethoxysilane (10%)<br>(weight ratio)  |

The quality of duplicated image on the printing plate precursor thus obtained was visually evaluated through a

With each of the lithographic printing plate precursors, the Bekk smoothness of the surface thereof was in a range

of from 250 to 300 (sec/10 ml), and the contact angle of the surface thereof with water was 0 degree.

Each of the lithographic printing plate precursor was subjected to plate-making and printing in the same manner as in Example 101. The printed matter obtained had clear images free from background stain in the non-image area similar to that obtained in Example 101. The press life of each lithographic printing plate was good as more than 10,000 sheets.

#### EXAMPLE 121

A lithographic printing plate precursor was prepared in the same manner as in Example 28 except for using 45 g of nickel hydroxide (average particle size: 40 nm) in place of 45 g of zinc oxide (Finex-50).

The Bekk smoothness of the surface of the lithographic printing plate precursor was 300 (sec/10 ml), and the contact angle of the surface with water was not more than 5 degrees.

The lithographic printing plate precursor was subjected to plate-making in the same manner as in Example 28. The image formed on the lithographic printing plate precursor was clear and free from distortion and blur in the accurate image portion such as fine lines and fine letters.

Using the printing plate thus obtained, printing was conducted in the same manner as in Example 101. The printed matter obtained had clear images free from background stain in the non-image area similar to that obtained in Example 101. The press life of the lithographic printing plate was good as more than 10,000 sheets.

#### EXAMPLE 201

A lithographic printing plate precursor was prepared in the same manner as in Example 1 except for using 100 g of barium titanate ( $\text{BaTiO}_3$ , average particle size: 0.6  $\mu\text{m}$ ) in place of 100 g of zinc oxide (Finex-50).

#### Comparative Example 201A

A lithographic printing plate precursor was prepared in the same manner as in Example 201 except for using 100 g of titanium oxide ( $\text{TiO}_2$ , average particle size: 0.3  $\mu\text{m}$ ) in place of 100 g of barium titanate.

The lithographic printing plate precursors prepared in Example 201 and Comparative Example 201A were subjected to evaluating their properties, respectively. The results obtained are shown in Table A-201 below.

TABLE A-201

|                                                                       | Example 201                                                                                                                                   | Comparative Example 201A                                                                                                           |
|-----------------------------------------------------------------------|-----------------------------------------------------------------------------------------------------------------------------------------------|------------------------------------------------------------------------------------------------------------------------------------|
| Surface Smoothness of Image-receiving Layer <sup>1)</sup> (sec/10 ml) | 310                                                                                                                                           | 270                                                                                                                                |
| Contact Angle with Water <sup>2)</sup> (degree)                       | 0                                                                                                                                             | 0                                                                                                                                  |
| Image Reproducibility <sup>3)</sup>                                   | neither blur nor distortion of fine lines and fine letters; shape of dot: true circle; true circle; sufficient density in solid image portion | neither blur nor distortion of fine lines and fine letters; shape of dot: true circle; insufficient density in solid image portion |

TABLE A-201-continued

|                          | Example 201                   | Comparative Example 201A |
|--------------------------|-------------------------------|--------------------------|
| Press Life <sup>4)</sup> | image portion<br>4,000 sheets | 1,000 sheets             |

10 The properties described in Table A-201 were evaluated in the following manner.

#### Surface Smoothness of Image-receiving Layer<sup>1)</sup>

A Bekk smoothness of the surface of the lithographic printing plate precursor was measured using a Bekk smoothness tester (manufactured by Kumagai Riko Co., Ltd.) under the condition of the air volume of 10 ml.

#### Contact Angle with Water<sup>2)</sup>

On the surface of the lithographic printing plate precursor was put 2  $\mu\text{l}$  of distilled water, and after a 30-second lapse at room temperature a contact angle of the lithographic printing plate precursor surface with water was measured using a surface contact angle meter (CA-D manufactured by Kyowa Kaimen Kagaku Co., Ltd.).

#### Image Reproducibility<sup>3)</sup>

A servo plotter (DA 8400 manufactured by Graphtech Co.) able to write in accordance with an output from a personal computer was converted so that an ink ejection head as shown in FIG. 4 was mounted on a pen plotter section, and the lithographic printing plate precursor described above was placed on a counter electrode positioned at a distance of 500  $\mu\text{m}$  from the ink ejection head.

40 Ink jet printing was performed on the lithographic printing plate precursor using Oil-Based Ink (IK-2) shown below to conduct image formation. Then, the printing plate precursor was heated by means of a Ricoh Fuser (Model 592 manufactured by Ricoh Co., Ltd.) so as to control the surface temperature of the printing plate precursor to 80° C. for one minute, thereby thoroughly fixing the ink image.

45 The image formed on the printing plate precursor was visually observed under an optical microscope of 200 magnifications.

#### <Preparation of Oil-Based Ink (IK-2)>

50 A mixed solution of 7 g of Dispersion Stabilizing Resin (PS-1) shown below, 100 g of vinyl acetate and 321 g of Isopar H was heated to a temperature of 75° C. under nitrogen gas stream with stirring. To the solution was added 1.5 g of 2,2'-azobis(isovaleronitrile) (abbreviated as AIVN) as a polymerization initiator, followed by reacting for 3 hours. Further, 1.0 g of AIVN was added to the reaction mixture, followed by reacting for 3 hours. Then, the temperature of the reaction mixture was raised to 100° C., followed by stirring for 2 hours, thereby distilling off the 55 unreacted vinyl acetate. After cooling the reaction mixture, it was passed through a nylon cloth of 200 mesh. The resulting white dispersion was a latex of good monodisperse.

sity having a polymerization rate of 93% and an average particle size of 0.42  $\mu\text{m}$ . The particle size was measured by CAPA-500 manufactured by Horiba Ltd.  
Dispersion Stabilizing Resin (PS-1)



A part of the above-described white dispersion was centrifuged at a rotation of  $1 \times 10^4$  r.p.m. for 60 minutes and the resin particles precipitated were collected and dried. A weight average molecular weight (Mw) of the resin particles was measured by a GPC method and calculated in terms of polystyrene. The weight average molecular weight (Mw) of the resin particles was  $2 \times 10^5$ , and a glass transition point (Tg) thereof was 38° C. The resulting resin particle was designated as Resin Particle (PL-2)

Ten grams of poly(dodecyl methacrylate), 10 g of Microlith Blue 4GT (manufactured by Ciba-Geigy Ltd.) and 80 g of Isopar G were placed in a paint shaker (manufactured by Toyo Seiki Seisakusho Corp.) together with glass beads and dispersed for 4 hours to obtain a fine dispersion of the blue pigment.

Twenty grams (as a solid basis) of Resin Particle (PL-2) described above, 7.5 g of the above-described blue-colored dispersion and 0.08 g of octadecene-maleic acid mono-octadecylamide copolymer were diluted with one liter of Isopar E, thereby obtaining blue-colored Oil-Based Ink (IK-2). Press Life<sup>4)</sup>

The image formation on the lithographic printing plate precursor and fixing of the image were conducted in the same manner as described in the image reproducibility<sup>3)</sup> above to prepare a lithographic printing plate.

The lithographic printing plate thus prepared was subjected to printing using as a printing machine, Oliver Model 94 manufactured by Sakurai Seisakusho Co., Ltd., as dampening water, a solution prepared by diluting EU-3 (manufactured by Fuji Photo Film Co., Ltd.) 50 times with water and black ink for offset printing.

A number of printed matter obtained without background stain and disappearance of fine lines and fine letters was determined as the press life.

As shown in Table A-201 above, the surface smoothness of the image-receiving layer was almost same in Example 201 and Comparative Example 201A. The contact angle with water was 0 degree in each example. This means that the surface has good hydrophilicity. With respect to the printing plate formed by plate-making in Example 201, neither blur nor distortion of fine lines and fine letters were observed, the density in the solid image portion was sufficiently high, and the dot image had true circular shape. On the contrary, the printing plate formed by plate-making in Comparative Example 201A had insufficient density in the solid image portion, although the reproducibility of fine lines and fine letters and the shape of dot were same as those in Example 201.

As a result of the printing 4,000 sheets of printed matter having clear images free from stain due to adhesion of printing ink were obtained in Example 201. In Comparative Example 201A, on the contrary, disappearance of the image area occurred after printing about 1,000 sheets, while stain in the non-image area was not observed.

#### EXAMPLE 202 TO 219

Each lithographic printing plate precursor was prepared in the same manner as in Example 201 except for using 100 g

of each of the compounds (the average particle size of each compound being in a range of from 0.03 to 2  $\mu\text{m}$ ) shown in Table B-201 below in place of 100 g of barium titanate.

With each of the lithographic printing plate precursors, the Bekk smoothness of the surface thereof was in a range of from 250 to 300 (sec/10 ml), and the contact angle of the surface thereof with water was 0 degree.

Each lithographic printing plate precursor was subjected to plate-making and printing in the same manner as in Example 201. The printed matter obtained had clear images free from background stain in the non-image area and blur and distortion of fine lines and fine letters. The press life of each lithographic printing plate was good as more than 4,000 sheets.

TABLE B-201

| Example | Double Oxide                                                              |
|---------|---------------------------------------------------------------------------|
| 202     | Magnesium silicate<br>(MgSiO <sub>3</sub> )                               |
| 203     | Cobalt silicate<br>(CoSiO <sub>4</sub> )                                  |
| 204     | Strontium titanate<br>(SrTiO <sub>3</sub> )                               |
| 205     | Zirconium titanate<br>(ZrO <sub>2</sub> .TiO <sub>2</sub> )               |
| 206     | Zinc titanate<br>(ZnTiO <sub>3</sub> )                                    |
| 207     | Barium zirconate<br>(BaZrO <sub>4</sub> )                                 |
| 208     | Lead stannate<br>(PbSnO <sub>3</sub> )                                    |
| 209     | Magnesium tungstate<br>(MgWO <sub>4</sub> )                               |
| 210     | Strontium vanadate<br>(SrV <sub>2</sub> O <sub>6</sub> )                  |
| 211     | Lead chromate<br>(PbCrO <sub>4</sub> )                                    |
| 212     | Basic lead chromate<br>(PbCrO <sub>4</sub> .PbO)                          |
| 213     | Strontium molybdate<br>(SrMoO <sub>4</sub> )                              |
| 214     | Nickel titanate<br>(NiTiO <sub>3</sub> )                                  |
| 215     | Aluminum tungstate<br>(Al <sub>2</sub> (WO <sub>4</sub> ) <sub>3</sub> )  |
| 216     | Zinc silicate<br>(ZnO.SiO <sub>2</sub> )                                  |
| 217     | Lead zirconate<br>(PbO.ZrO <sub>2</sub> )                                 |
| 218     | Aluminum molybdate<br>(Al <sub>2</sub> (MoO <sub>4</sub> ) <sub>3</sub> ) |
| 219     | Calcium zirconate<br>(CaZrO <sub>3</sub> )                                |

#### EXAMPLE 220

<Preparation of Direct Drawing Type Lithographic Printing Plate Precursor>

A composition having the following component was placed in a paint shaker (manufactured by Toyo Seiki Seisakusho Corp.) together with glass beads and dispersed for 30 minutes at room temperature. Then, the glass beads were removed by filtration to obtain a dispersion.

|                                                                                                 |       |
|-------------------------------------------------------------------------------------------------|-------|
| Strontium titanate (SrTiO <sub>3</sub> , average particle size: 60 nm)                          | 45 g  |
| 10% By weight aqueous solution of gelatin                                                       | 100 g |
| 20% By weight aqueous dispersion of colloidal silica (Snowtex C manufactured by Nissan Chemical | 25 g  |

-continued

|                                                                                                                                               |       |    |  |
|-----------------------------------------------------------------------------------------------------------------------------------------------|-------|----|--|
| Industries, Ltd.)                                                                                                                             |       |    |  |
| Tetraethoxysilane                                                                                                                             | 30 g  | 5  |  |
| Fluorinated alkyl ester (FC-430 manufactured by 3M Co.)                                                                                       | 0.2 g |    |  |
| Hardening agent                                                                                                                               | 0.5 g |    |  |
| CH <sub>2</sub> =CHSO <sub>2</sub> CH <sub>2</sub> CONH(CH <sub>2</sub> ) <sub>3</sub> NHCOCH <sub>2</sub> SO <sub>2</sub> CH=CH <sub>2</sub> |       |    |  |
| 1N Hydrochloric acid                                                                                                                          | 2 g   |    |  |
| Solvent mixture of water and ethanol (1/1 in weight ratio)                                                                                    | 200 g | 10 |  |

On a support for ELP-2X Type Master, the coating composition prepared above was coated by means of a wire bar, set to touch and then heated at 110° C. for 30 minutes to form an image-receiving layer having a coating amount of 6 g/m<sup>2</sup>. Thus, a lithographic printing plate precursor was prepared.

The Bekk smoothness of the surface of the lithographic printing plate precursor was 450 (sec/10 ml), and the contact angle of the surface with water was 0 degree.

The lithographic printing plate precursor was subjected to plate-making in the same manner as in Example 19.

The image formed on the lithographic printing plate precursor was observed under an optical microscope of 200 magnifications to evaluate its image quality. The image formed was clear and free from blur and disappearance of fine lines and fine letters.

Then, the lithographic printing plate thus-prepared was subjected to printing in the same manner as in Example 19.

The 10th printed matter was picked up in the course of printing, and the printed image thereon was evaluated by visual observation using a magnifier of 20 magnifications. The observation result indicated that the non-image area was free from background stain due to adhesion of the printing ink and the uniformity of the solid image portion was good. Further, the printed matter was observed under an optical microscope of 200 magnifications. According to the observation, neither sharpening nor disappearance were found in the area of fine lines and fine letters, and the image quality of printed matter was good.

As a result of continuing the printing procedure, more than 5,000 sheets of printed matter having image quality equal to that of the 10th print were obtained.

## EXAMPLE 221

A lithographic printing plate precursor was prepared in the same manner as in Example 20 except for using a composition for image-receiving layer having the following component in place of the composition for image-receiving layer used in Example 20.

|                                                                                                        |       |
|--------------------------------------------------------------------------------------------------------|-------|
| Magnesium zirconate (average particle size: 1.2 μm)                                                    | 80 g  |
| 10% By weight aqueous solution of starch (Penon ZP-2 manufactured by Nichiden Chemical Co., Ltd.)      | 300 g |
| Clay                                                                                                   | 10 g  |
| Tetrapropoxysilane                                                                                     | 40 g  |
| Methyltrimethoxysilane                                                                                 | 3 g   |
| Alumina sol (520 manufactured by Nissan Chemical Industries, Ltd.; average particle size: 10 to 20 nm) | 10 g  |
| Ethanol                                                                                                | 110 g |
| 1N Hydrochloric acid                                                                                   | 5 g   |
| Water                                                                                                  | 150 g |

15

The Bekk smoothness of the surface of the lithographic printing plate precursor was 150 (sec/10 ml), and the contact angle of the surface with water was 0 degree.

The lithographic printing plate precursor was subjected to plate-making in the same manner as in Example 20.

The quality of duplicated image on the printing plate precursor thus obtained was visually evaluated through a magnifier of 20 magnifications, and it was found that the image quality was good. Specifically, the plate-making image formed by transfer of dry toner from the laser printer had no disappearance of fine lines and fine letters and uniform solid image portion, and unevenness of toner transfer was not observed at all. Although, the background stain due to scattering of toner was slightly occurred in the non-image area, it was practically acceptable.

The lithographic printing plate precursor was subjected to plate-making in the same manner as described above. The lithographic printing plate thus prepared was then subjected to printing in the same manner as in Example 20. The 10th sheet was picked up in the course of printing, and the printed image thereon was visually evaluated for its image quality (background stain and uniformity in solid image portion) through a magnifier of 20 magnifications. The image quality was excellent.

As a result of continuing the printing procedure, 4,000 sheets of printed matter having image quality equal to that of the 10th print were obtained.

## EXAMPLE 222 TO 228

Lithographic printing plate precursors were prepared in the same manner as in Example 201 except for using the organic polymer and the silane compound shown in Table C-201 below in place of polyvinyl alcohol (PVA 117) and tetraethoxysilane, respectively.

TABLE C-201

| Example | Organic Polymer                                                                         | Silane Compound (weight ratio)                                                    |
|---------|-----------------------------------------------------------------------------------------|-----------------------------------------------------------------------------------|
| 222     | Polyvinylpyrrolidone                                                                    | Triethoxysilane (20%)<br>Tetramethoxysilane (80%)                                 |
| 223     | Propyleneoxide-modified starch (PENON HV-2 manufactured by Nichiden Chemical Co., Ltd.) | Tetra(2-methoxyethoxy)titanium (5%)                                               |
| 224     | Hydroxypropylated starch (PENON LD-1 manufactured by Nichiden Chemical Co., Ltd.)       | Tetrabutoxysilane (95%)<br>Octyltrimethoxysilane (1%)<br>Tetrapropoxysilane (99%) |
| 225     | N-Methylolacrylamide/methyl acrylate (85/15 in weight ratio) copolymer                  | 3-Hydroxypropyltrimethoxysilane (5%)<br>Tetraethoxysilane (95%)                   |

TABLE C-201-continued

| Example | Organic Polymer                                                                        | Silane Compound (weight ratio)                                      |
|---------|----------------------------------------------------------------------------------------|---------------------------------------------------------------------|
| 226     | Polyethylene glycol 20,000<br>(manufactured by Wako Pure<br>Chemical Industries, Ltd.) | Methyltrimethoxysilane (2%)<br>Tetraethoxysilane (98%)              |
| 227     | Polyvinyl alcohol (PVA 405<br>manufactured by Kuraray Co.,<br>Ltd.)                    | 2-Carboxyethyltrimethoxy-<br>silane (5%)<br>Tetraethoxysilane (95%) |
| 228     |                                                                                        | Tetraethoxysilane (90%)<br>3-Sulfopropyltrimethoxy-<br>silane (10%) |

With each of the lithographic printing plate precursors, the Bekk smoothness of the surface thereof was in a range of from 250 to 300 (sec/10 ml), and the contact angle of the surface thereof with water was 0 degree.

Each of the lithographic printing plate precursor was subjected to plate-making and printing in the same manner as in Example 101. The printed matter obtained had clear images free from background stain in the non-image area similar to that obtained in Example 101. The press life of each lithographic printing plate was good as more than 3,000 sheets.

#### EXAMPLE 229

A lithographic printing plate precursor was prepared in the same manner as in Example 28 except for using 45 g of zinc zirconate (average particle size: 1.3  $\mu\text{m}$ ) in place of 45 g of zinc oxide (Finex-50).

The Bekk smoothness of the surface of the lithographic printing plate precursor was 300 (sec/10 ml), and the contact angle of the surface with water was not more than 5 degrees.

The lithographic printing plate precursor was subjected to plate-making using an electrostatic ejection type ink jet recording device as described in WO 93/11866 and Oil-Based Ink (IK-2) described in Example 201. The image formed on the lithographic printing plate precursor was clear and free from distortion and blur in the accurate image portion such as fine lines and fine letters.

Using the printing plate thus obtained, printing was conducted in the same manner as in Example 201. The printed matter obtained had clear images free from background stain in the non-image area similar to that obtained in Example 201. The press life of the lithographic printing plate was good as more than 5,000 sheets.

While the invention has been described in detail and with reference to specific examples thereof, it will be apparent to one skilled in the art that various changes and modifications can be made therein without departing from the spirit and scope thereof.

What is claimed is:

1. A direct drawing lithographic printing plate precursor comprising a water-resistant support having provided thereon an image-receiving layer comprising inorganic particles and a binder resin,

wherein said inorganic particles comprises at least one kind of particles selected from:

(1) metal oxide particles having an average particle size of from 0.01 to 5  $\mu\text{m}$  and comprising a metal atom selected from Mg, Ba, Ge, Sn, Zn, Pb, La, Zr, V, Cr, Mo, W, Mn, Co, Ni and Cu;

(ii) metal hydroxide particles having an average particle size of from 0.01 to 5  $\mu\text{m}$ , said metal hydroxide being represented by the following formula (I):



wherein M Represents a metal atom selected from Mg, Ba, Al, Ti, Zn, Cu, Ni, Sn, Co, Ge, Fe and La, and x represents a valence of said metal M; and

(iii) double oxide particles having an average particle size of from 0.01 to 5  $\mu\text{m}$  and comprising at least one metal atom selected from Mg, Al, Si, Ti, Zr, Cr, V, Mo, Sn, W and Nb, and

wherein said binder resin comprises a complex comprising: a resin containing a siloxane bond in which a silicon atom is connected with an oxygen atom; and an organic polymer containing a group capable of forming a hydrogen bond with said resin containing the siloxane bond.

2. The direct drawing lithographic printing plate precursor as claimed in claim 1, wherein said resin containing the siloxane bond is a polymer formed by a hydrolysis polymerization condensation reaction of at least one silane compound represented by the following formula (II):



wherein  $\text{R}^0$  represents a hydrogen atom, a hydrocarbon group or a heterocyclic group; Y represents a hydrogen atom, a halogen atom,  $-\text{OR}^1$ ,  $-\text{OCOR}^2$  or  $-\text{N}(\text{R}^3)$  (wherein  $\text{R}^1$  and  $\text{R}^2$  each represents a hydrocarbon group, and  $\text{R}^3$   $\text{R}^4$ , which may be the same or different, each represents a hydrogen atom or a hydrocarbon group); and n represents 0, 1 or 2, provided that the Si atom is not connected to three or more hydrogen atoms.

3. The direct drawing lithographic printing plate precursor as claimed in claim 1, wherein said image-receiving layer has a surface smoothness of not less than 30 seconds/10 ml in terms of a Bekk smoothness.

4. The direct drawing lithographic printing plate precursor as claimed in claim 1, wherein said organic polymer containing the group capable of forming a hydrogen bond with said resin containing the siloxane bond is a polymer containing at least one member selected from the group consisting of an amido bond, a urethane bond, a ureido bond and a hydroxy group.

5. The direct drawing lithographic printing plate precursor as claimed in claim 4, wherein said organic polymer is: an amide resin having an  $-\text{N}(\text{R}^{11})\text{CO}-$  or  $-\text{N}(\text{R}^{11})\text{SO}_2-$  bond wherein  $\text{R}^{11}$  represents a hydrogen atom, a hydrocarbon group or a heterocyclic group; a ureide resin having an

45

—NHCONH— bond; or a urethane resin having an —NHCOO— bond.

6. The direct drawing lithographic printing plate precursor as claimed in claim 4, wherein said organic polymer is a polymer containing a repeating unit represented by the following formula (III):



wherein  $Z^1$  represents —CO—, —CS— or —SO<sub>2</sub>—;  $R^{20}$  represents a hydrogen atom, a hydrocarbon group or a heterocyclic group;  $r^1$  represents a hydrogen atom or an alkyl group having from 1 to 6 carbon atoms, and a plurality of  $r^1$  groups may be the same or different; and  $p$  represents an integer of 2 or 3.

7. The direct drawing lithographic printing plate precursor as claimed in claim 1, wherein said complex has a weight ratio of the siloxane polymer/organic polymer of from 10/90 to 90/10.

8. The direct drawing lithographic printing plate precursor as claimed in claim 1, wherein said image-receiving layer has a surface of high dense protrusions.

9. The direct drawing lithographic printing plate precursor as claimed in claim 8, wherein said image-receiving layer

46

has an average surface center roughness (SRa) defined in ISO-468 of from 1.3 to 3.5  $\mu\text{m}$ , and an average wavelength (S $\lambda$ a) of not more than 50  $\mu\text{m}$ .

10. The direct drawing lithographic printing plate precursor as claimed in claim 1, wherein said image-receiving layer has a thickness of from 0.2 to 10  $\mu\text{m}$ .

11. The direct drawing lithographic printing plate precursor as claimed in claim 1, wherein said water-resistant support has a surface smoothness of not less than 300 seconds/10 ml in terms of a Bekk smoothness.

12. The direct drawing lithographic printing plate precursor as claimed in claim 1, wherein said water-resistant support has specific electric resistance of from 10<sup>4</sup> to 10<sup>13</sup>  $\Omega\text{cm}$ .

13. The direct drawing lithographic printing plate precursor as claimed in claim 1, wherein said inorganic particles comprise said metal oxide particles (i).

14. The direct drawing lithographic printing plate precursor as claimed in claim 1, wherein the inorganic particles comprise said metal hydroxide particles (ii).

15. The direct drawing lithographic printing plate precursor as claimed in claim 1, wherein the inorganic particles comprise said double oxide particles (iii).

\* \* \* \* \*